



(51) **Int. Cl.**  
*H01T 13/41* (2006.01)  
*F02P 11/00* (2006.01)

(56) **References Cited**

FOREIGN PATENT DOCUMENTS

|    |              |         |       |            |
|----|--------------|---------|-------|------------|
| JP | S52-125946 A | 10/1977 | ..... | H01T 13/00 |
| JP | S52-125947 A | 10/1977 | ..... | H01T 13/00 |
| JP | S54-151736 A | 11/1979 | ..... | H01T 13/02 |
| JP | S54-151737 A | 11/1979 | ..... | H01T 13/02 |
| JP | S56-172914 U | 12/1981 | ..... | H01F 17/04 |
| JP | S61-104580 A | 5/1986  | ..... | H01T 13/20 |
| JP | S61-135079 A | 6/1986  | ..... | H01T 13/20 |
| JP | S61-208768 A | 9/1986  | ..... | H01T 13/20 |
| JP | S61-230281 A | 10/1986 | ..... | H01C 7/00  |
| JP | S61-284903 A | 12/1986 | ..... | H01C 17/00 |
| JP | S62-150681 A | 7/1987  | ..... | H01T 13/20 |
| JP | H02-284374 A | 11/1990 | ..... | F02P 13/00 |

FIG. 1



FIG.2



FIG.3



FIG.4



FIG.5



FIG. 6



FIG. 7



**1**  
**SPARK PLUG**

RELATED APPLICATIONS

This application is a National Stage of International Application No. PCT/JP2014/084392 filed Dec. 25, 2014, which claims the benefit of Japanese Patent Application No. 2013-266957, filed Dec. 25, 2013.

FIELD OF THE INVENTION

This disclosure relates to a spark plug.

BACKGROUND OF THE INVENTION

Conventionally, a spark plug has been used in an internal combustion engine. Technology, by which a resistor is provided in a through hole of an insulator so as to suppress occurrence of electromagnetic noise induced by ignition, has been proposed. Technology, by which a magnetic substance is provided in the through hole of the insulator, has also been proposed.

The fact is that enough study regarding the suppression of electromagnetic noise by the magnetic substance has not been made.

This disclosure discloses technology by which the occurrence of electromagnetic noise can be suppressed by a magnetic substance.

SUMMARY OF THE INVENTION

This disclosure discloses the following application examples and the like.

APPLICATION EXAMPLE 1

In accordance with a first aspect of the present invention, there is provided a spark plug comprising:  
an insulator having a through hole extending in a direction of an axial line;  
a center electrode, at least a part of which is inserted into a leading end side of the through hole;  
a terminal metal fixture, at least a part of which is inserted into a rear end side of the through hole; and  
a connection portion connecting the center electrode and the terminal metal fixture together in the through hole, wherein the connection portion includes:  
a resistor; and  
a magnetic substance structure including a magnetic substance and a conductor and being disposed on a leading end side or a rear end side of the resistor while being positioned away from the resistor, and wherein, among the resistor and the magnetic substance structure, when a member disposed on a leading end side is defined as a first member and a member disposed on a rear end side is defined as a second member, the connection portion further includes:  
a first conductive sealing portion that is disposed on a leading end side of the first member and is in contact with the first member;  
a second conductive sealing portion that is disposed between the first member and the second member and is in contact with the first member and the second member; and  
a third conductive sealing portion that is disposed on a rear end side of the second member and is in contact with the second member.

**2**

In this configuration, it is possible to suppress occurrence of an electrical contact failure at both ends of the resistor and an electrical contact failure at both ends of the magnetic substance structure by using the first, the second, and the third conductive sealing portions. Accordingly, it is possible to appropriately suppress electromagnetic noise by using both the resistor and the magnetic substance structure.

APPLICATION EXAMPLE 2

10 In accordance with a second aspect of the present invention, there is provided a spark plug as described above, wherein an electrical resistance between a leading end and a rear end of the magnetic substance structure is less than or equal to 3 kΩ.  
15 In this configuration, it is possible to suppress heat generation of the magnetic substance structure. Accordingly, it is possible to suppress the occurrence of a failure (for example, alteration of the magnetic substance) induced by heat generation of the magnetic substance structure.

APPLICATION EXAMPLE 3

20 In accordance with a third aspect of the present invention, there is provided a spark plug as described above, wherein the electrical resistance between the leading end and the rear end of the magnetic substance structure is less than or equal to 1 kΩ.

25 In this configuration, it is possible to further suppress heat generation of the magnetic substance structure. Accordingly, it is possible to further suppress the occurrence of a failure (for example, alteration of the magnetic substance) induced by heat generation of the magnetic substance structure.

APPLICATION EXAMPLE 4

30 In accordance with a fourth aspect of the present invention, there is provided a spark plug as described above, wherein the conductor includes a spiral coil surrounding at least a part of an outer circumference of the magnetic substance, and wherein an electrical resistance of the coil is less than an electrical resistance of the magnetic substance.

35 In this configuration, it is possible to appropriately suppress electromagnetic noise while suppressing heat generation of the magnetic substance using the coil.

APPLICATION EXAMPLE 5

40 In accordance with a fifth aspect of the present invention, there is provided a spark plug as described above, wherein the conductor includes a conductive portion penetrating through the magnetic substance in the direction of the axial line.

45 In this configuration, it is possible to appropriately suppress electromagnetic noise while improving durability.

APPLICATION EXAMPLE 6

50 In accordance with a sixth aspect of the present invention, there is provided a spark plug as described above, wherein the magnetic substance structure is disposed on the rear end side of the resistor.

55 In this configuration, it is possible to appropriately suppress electromagnetic noise.

APPLICATION EXAMPLE 7

60 In accordance with a seventh aspect of the present invention, there is provided a spark plug as described above,

wherein the connection portion further includes a covering portion that covers at least a part of an outer surface of the magnetic substance structure while being interposed between the magnetic substance structure and the insulator.

In this configuration, it is possible to suppress direct contact between the insulator and the magnetic substance structure.

#### APPLICATION EXAMPLE 8

In accordance with an eighth aspect of the present invention, there is provided a spark plug as described above, wherein the magnetic substance is made of a ferromagnetic material containing an iron oxide.

In this configuration, it is possible to appropriately suppress electromagnetic noise.

#### APPLICATION EXAMPLE 9

In accordance with a ninth aspect of the present invention, there is provided a spark plug as described above, wherein the ferromagnetic material is a spinel type ferrite.

In this configuration, it is possible to easily suppress electromagnetic noise.

#### APPLICATION EXAMPLE 10

In accordance with a tenth aspect of the present invention, there is provided a spark plug as described above, wherein the magnetic substance is a NiZn ferrite or a MnZn ferrite.

In this configuration, it is possible to appropriately suppress electromagnetic noise.

#### APPLICATION EXAMPLE 11

In accordance with an eleventh aspect of the present invention, there is provided a spark plug as described above, wherein the magnetic substance structure contains:

- (1) a conductive substance as the conductor;
- (2) an iron-containing oxide as the magnetic substance; and
- (3) a ceramic containing at least one of silicon (Si), boron (B), and phosphorous (P),

wherein, in a cross-section of the magnetic substance structure including the axial line, when a target region is defined as a rectangular region having the axial line as a center line, a side of 2.5 mm in a direction perpendicular to the axial line, and a side of 5.0 mm in the direction of the axial line,

a region of the iron-containing oxide includes a plurality of grain-shaped regions in the target region,

at least a part of an edge of each of the plurality of grain-shaped regions is covered with the conductive substance in the target region, and

when a coverage is defined as a proportion of a length of a portion of the edge of the grain-shaped region covered with the conductive substance to an entire length of the edge of the grain-shaped region, an average value of the coverage of the plurality of grain-shaped regions is greater than or equal to 50% in the target region.

In this configuration, since the magnetic substance structure has specific properties, it is possible to appropriately suppress noise.

#### APPLICATION EXAMPLE 12

In accordance with a twelfth aspect of the present invention, there is provided a spark plug as described above,

wherein, in the target region in the cross-section of the magnetic substance structure, a porosity of a remainder of the target region other than the region of the iron-containing oxide is less than or equal to 5%.

In this configuration, it is possible to appropriately suppress electromagnetic noise.

#### APPLICATION EXAMPLE 13

In accordance with a thirteenth aspect of the present invention, there is provided a spark plug as described above, wherein, in the target region in the cross-section of the magnetic substance structure, a total number of grain-shaped regions, an area of which is the same as an area of a circle with a diameter in a range of 400  $\mu\text{m}$  or greater and 1,500  $\mu\text{m}$  or less, is greater than or equal to 6.

In this configuration, it is possible to further appropriately suppress electromagnetic noise.

#### APPLICATION EXAMPLE 14

In accordance with a fourteenth aspect of the present invention, there is provided a spark plug as described above, wherein, in the target region in the cross-section of the magnetic substance structure, a minimum thickness of the conductive substance covering the edge of the grain-shaped region is 1  $\mu\text{m}$  or greater and 25  $\mu\text{m}$  or less.

In this configuration, it is possible to further appropriately suppress electromagnetic noise.

#### APPLICATION EXAMPLE 15

In accordance with a fifteenth aspect of the present invention, there is provided a spark plug as described above, further comprising:

- a metal shell disposed on a radial circumference of the insulator,
- wherein the magnetic substance structure is disposed on the rear end side of the resistor, and
- wherein a rear end of the magnetic substance structure is positioned closer to the rear end side than a rear end of the metal shell.

In this configuration, it is possible to further appropriately suppress electromagnetic noise.

#### APPLICATION EXAMPLE 16

In accordance with a sixteenth aspect of the present invention, there is provided a spark plug comprising:

- an insulator having a through hole extending in a direction of an axial line;
- a center electrode, at least a part of which is inserted into a leading end side of the through hole;
- a terminal metal fixture, at least a part of which is inserted into a rear end side of the through hole; and
- a connection portion connecting the center electrode and the terminal metal fixture together in the through hole,

wherein the connection portion includes a magnetic substance structure including a magnetic substance and a conductor,

wherein the magnetic substance structure contains:

- (1) a conductive substance as the conductor;
- (2) an iron-containing oxide as the magnetic substance; and
- (3) a ceramic containing at least one of silicon (Si), boron (B), and phosphorous (P),

wherein, in a cross-section of the magnetic substance structure including the axial line, when a target region is defined as a rectangular region having the axial line as a center line, a side of 2.5 mm in a direction perpendicular to the axial line, and a side of 5.0 mm in the direction of the axial line,

a region of the iron-containing oxide includes a plurality of grain-shaped regions in the target region,

at least a part of an edge of each of the plurality of grain-shaped regions is covered with the conductive substance in the target region, and

when a coverage is defined as a proportion of a length of a portion of the edge of the grain-shaped region covered with the conductive substance to an entire length of the edge of the grain-shaped region, an average value of the coverage of the plurality of grain-shaped regions is greater than or equal to 50% in the target region.

In this configuration, since the magnetic substance structure has specific properties, it is possible to appropriately suppress electromagnetic noise.

One or more application examples arbitrarily selected from Application Examples 1 to 15 may be combined to Application Example 16.

#### BRIEF DESCRIPTION OF DRAWINGS

FIG. 1 is a cross-sectional view of a spark plug 100 in a first embodiment.

FIG. 2 is a cross-sectional view of a spark plug 100b in a second embodiment.

FIG. 3 is a cross-sectional view of a spark plug 100c in a reference example.

FIG. 4 is a cross-sectional view of a spark plug 100d in a third embodiment.

FIG. 5 shows views illustrating a magnetic substance structure 200d.

FIG. 6 is a partial enlarged view of the cross-sectional view illustrated in FIG. 4.

FIG. 7 is a cross-sectional view of a spark plug 100e in a fourth embodiment.

#### DETAILED DESCRIPTION OF THE PREFERRED EMBODIMENTS

##### A. First Embodiment

###### A-1. Configuration of Spark Plug:

FIG. 1 is a cross-sectional view of a spark plug 100 in a first embodiment. An illustrated line CL is a center axis of the spark plug 100. The illustrated cross-section is a cross-section including the center axis CL. Hereinafter, the center axis CL may be referred to as an "axial line CL", and a direction parallel with the center axis CL may be referred to as a "direction of the axial line CL", or simply as an "axial direction". A radial direction of a circle centered around the center axis CL may be simply referred to as a "radial direction", and a circumferential direction of the circle centered around the center axis CL may be referred to as a "circumferential direction". In FIG. 1, among the directions parallel with the center axis CL, a downward direction may be referred to as a leading end direction D1, and an upward direction may be referred to as a rear end direction D2. The leading end direction D1 is a direction running from a terminal metal fixture 40 (to be described later) toward electrodes 20 and 30. In FIG. 1, the leading end direction D1 side is referred to as the leading end side of the spark plug

100, and the rear end direction D2 side is referred to as the rear end side of the spark plug 100.

The spark plug 100 includes an insulator 10 (may be referred to as a "ceramic insulator 10"); the center electrode 20; the ground electrode 30; the terminal metal fixture 40; a metal shell 50; a first conductive sealing portion 60; a resistor 70; a second conductive sealing portion 75; a magnetic substance structure 200; a covering portion 290; a third conductive sealing portion 80; a leading end side packing 8; talc 9; a first rear end-side packing 6; and a second rear end-side packing 7.

The insulator 10 is a substantially tubular member which extends along the center axis CL and has a through hole 12 (may be referred to as an "axial hole 12") penetrating through the insulator 10. The insulator 10 is made of alumina by firing (another insulating material may also be adopted). The insulator 10 includes a leg portion 13; a first reduced outer diameter portion 15; a leading end side trunk portion 17; a flanged portion 19; a second reduced outer diameter portion 11; and a rear end-side trunk portion 18, which line up sequentially from the leading end side toward the rear end side.

The flanged portion 19 is a portion of the insulator 10 which has the maximum outer diameter. An outer diameter 25 of the first reduced outer diameter portion 15 positioned closer to the leading end side than the flanged portion 19 is gradually reduced from the rear end side toward the leading end side. A reduced inner diameter portion 16 is formed in the vicinity of the first reduced outer diameter portion 15 of the insulator 10 (the leading end side trunk portion 17 in the example illustrated in FIG. 1), and an inner diameter of the reduced inner diameter portion 16 is gradually reduced from the rear end side toward the leading end side. An outer diameter of the second reduced outer diameter portion 11 30 positioned closer to the rear end side than the flanged portion 19 is gradually reduced from the leading end side toward the rear end side.

The center electrode 20 is inserted into a leading end side of the through hole 12 of the insulator 10. The center electrode 20 is a bar-shaped member which extends along the center axis CL. The center electrode 20 includes an electrode base member 21 and a core member 22 embedded in the electrode base member 21. For example, the electrode base member 21 is made of Inconel ("INCONEL" is registered trademark) that is an alloy containing nickel as a main component. The core member 22 is made of a material (for example, an alloy containing copper) having a coefficient of thermal conductivity greater than that of the electrode base member 21.

With focus given to an outer shape of the center electrode 20, the center electrode 20 includes a leg portion 25 formed at the end of the center electrode 20 on the leading end direction D1 side; a flanged portion 24 provided on the rear end side of the leg portion 25; and a head portion 23 provided on the rear end side of the flanged portion 24. The head portion 23 and the flanged portion 24 are disposed in the through hole 12, and the surface of the flanged portion 24 on the leading end direction D1 side is supported by the reduced inner diameter portion 16 of the insulator 10. A leading end side portion of the leg portion 25 is positioned on the leading end side of the insulator 10, and is exposed to the outside from the through hole 12.

The terminal metal fixture 40 is inserted into the rear end side of the through hole 12 of the insulator 10. The terminal metal fixture 40 is made of a conductive material (metal such as low-carbon steel). An anti-corrosion metal layer may be formed on the surface of the terminal metal fixture 40. For

example, a Ni layer may be formed by plating. The terminal metal fixture 40 includes a flange portion 42; a cap installation portion 41 that is formed to a portion of the terminal metal fixture 40 positioned closer to the rear end side than the flanged portion 42; and a leg portion 43 that is formed to a portion of the terminal metal fixture 40 positioned closer to the leading end side than the flanged portion 42. The cap installation portion 41 is positioned on the rear end side of the insulator 10, and is exposed to the outside from the through hole 12. The leg portion 43 is inserted into the through hole 12 of the insulator 10.

The resistor 70 suppressing electrical noise is disposed in the through hole 12 of the insulator 10 while being interposed between the terminal metal fixture 40 and the center electrode 20. The resistor 70 is made of a composite containing glass particles (for example,  $B_2O_3-SiO_2$  based glass) as a main component, and containing ceramic particles (for example,  $ZrO_2$ ) and a conductive material (for example, carbon particles) in addition to the glass.

The magnetic substance structure 200 suppressing electrical noise is disposed in the through hole 12 of the insulator 10 while being interposed between the resistor 70 and the terminal metal fixture 40. On the right side of FIG. 1, a perspective view of the magnetic substance structure 200 covered with the covering portion 290 and a perspective view of the magnetic substance structure 200 from which the covering portion 290 is removed are illustrated. The magnetic substance structure 200 includes a magnetic substance 210 and a conductor 220.

The magnetic substance 210 is a member that has a shape of a substantially circular column having the center axis CL as the center. For example, the magnetic substance 210 is made of a ferromagnetic material containing iron oxide. Spinel-type ferrite, hexagonal ferrite, and the like may be adopted as the ferromagnetic material containing iron oxide.  $NiZn$  (nickel-zinc) ferrite,  $MnZn$  (manganese-zinc) ferrite,  $CuZn$  (copper-zinc) ferrite, and the like may be adopted as the spinel-type ferrite.

The conductor 220 is a spiral coil surrounding the outer circumference of the magnetic substance 210. The conductor 220 is made of a metal wire, for example, an alloy wire material containing nickel and chromium as main components. The conductor 220 is wrapped around the magnetic substance 210, and extends from the vicinity of the end of the magnetic substance 210 on the leading end direction D1 side to the vicinity of the end of the magnetic substance 210 on the rear end direction D2 side.

The first conductive sealing portion 60 is disposed between the resistor 70 and the center electrode 20 in the through hole 12 while being in contact with the resistor 70 and the center electrode 20. The second conductive sealing portion 75 is disposed between the resistor 70 and the magnetic substance structure 200 while being in contact with the resistor 70 and the magnetic substance structure 200. The third conductive sealing portion 80 is disposed between the magnetic substance structure 200 and the terminal metal fixture 40 while being in contact with the magnetic substance structure 200 and the terminal metal fixture 40. The sealing portions 60, 75 and 80 contain similar glass particles as those of the resistor 70 and metal particles (Cu, Fe, and the like).

The center electrode 20 is electrically connected to the terminal metal fixture 40 via the resistor 70, the magnetic substance structure 200, and the sealing portions 60, 75, and 80. That is, the first conductive sealing portion 60, the resistor 70, the second conductive sealing portion 75, the magnetic substance structure 200, and the third conductive

sealing portion 80 form a conductive path through which the center electrode 20 is electrically connected to the terminal metal fixture 40. It is possible to stabilize the contact resistance between the members 20, 60, 70, 75, 200, 80 and 40 stacked on top of each other, and to stabilize the electrical resistance value between the center electrode 20 and the terminal metal fixture 40 by using the conductive sealing portions 60, 75, and 80. Hereinafter, all of a plurality of members 60, 70, 75, 200, 290 and 80, which are disposed in the through hole 12 and connect the center electrode 20 and the terminal metal fixture 40 together, may be referred to as a "connection portion 300".

In FIG. 1, a position 72 (may be referred to as a "rear end position 72") of the end of the resistor 70 on the rear end direction D2 side is illustrated. With respect to the through hole 12 of the insulator 10, an inner diameter of a portion disposed on the rear end direction D2 side of the rear end position 72 is slightly larger than an inner diameter of a portion disposed on the leading end direction D1 side of the rear end position 72 (particularly, a portion accommodating the first conductive sealing portion 60 and the resistor 70). However, both inner diameters may be the same.

The outer circumferential surface of the magnetic substance structure 200 is covered with the covering portion 290. The covering portion 290 is a tubular member covering the outer circumference of the magnetic substance structure 200. The covering portion 290 is interposed between an inner circumferential surface 10i of the insulator 10 and an outer circumferential surface of the magnetic substance structure 200. The covering portion 290 is made of glass (for example, borosilicate glass). During the operation of an internal combustion engine (not illustrated) equipped with the spark plug 100, vibration is transmitted from the internal combustion engine to the spark plug 100. The vibration may cause a positional offset between the insulator 10 and the magnetic substance structure 200. However, in the spark plug 100 according to the first embodiment, the covering portion 290 disposed between the insulator 10 and the magnetic substance structure 200 absorbs vibration, and thus the positional offset between the insulator 10 and the magnetic substance structure 200 can be suppressed.

The metal shell 50 is a substantially tubular member which extends along the center axis CL and has a through hole 59 penetrating through the metal shell 50. The metal shell 50 is made of low-carbon steel (another conductive material (for example, a metal material) may also be adopted). An anti-corrosion metal layer may be formed on the surface of the metal shell 50. For example, a Ni layer may be formed by plating. The insulator 10 is inserted into the through hole 59 of the metal shell 50, and the metal shell 50 is fixed to the outer circumference of the insulator 10. The leading end of the insulator 10 (in the embodiment, a leading end side portion of the leg portion 13) is exposed to the outside at the leading end side of the through hole 59 of the metal shell 50. The rear end (in the embodiment, a rear end-side portion of the rear end-side trunk portion 18) of the insulator 10 is exposed to the outside on the rear end side of the through hole 59 of the metal shell 50.

The metal shell 50 includes a trunk portion 55; a seat portion 54; a deformed portion 58; a tool engagement portion 51; and a crimped portion 53 which line up sequentially from the leading end side toward the rear end side. The seat portion 54 is a flange-like portion. The trunk portion 55 positioned on the leading end direction D1 side of the seat portion 54 has an outer diameter smaller than that of the seat portion 54. A screw portion 52 is formed in the outer circumferential surface of the trunk portion 55, and is

screwed into an attachment hole of an internal combustion engine (for example, a gasoline engine). An annular gasket 5 is fitted into the gap between the seat portion 54 and the screw portion 52, and is formed by folding a metal plate.

The metal shell 50 includes a reduced inner diameter portion 56 disposed closer to the leading end direction D1 side than the deformed portion 58. The inner diameter of the reduced inner diameter portion 56 is gradually reduced from the rear end side toward the leading end side. The leading end side packing 8 is interposed between the reduced inner diameter portion 56 of the metal shell 50 and the first reduced outer diameter portion 15 of the insulator 10. The leading end side packing 8 is a steel O-ring (another material (for example, metal material such as copper) may also be adopted).

The deformed portion 58 of the metal shell 50 is deformed in such a way that a center portion of the deformed portion 58 protrudes outward (a direction away from the center axis CL) in the radial direction. The tool engagement portion 51 is provided on the rear end side of the deformed portion 58. The tool engagement portion 51 is formed to have a shape (for example, a shape of a hexagonal column) so that a spark plug wrench can be engaged with the tool engagement portion 51. The crimped portion 53 is provided on the rear end side of the tool engagement portion 51, and has a thickness thinner than that of the tool engagement portion 51. The crimped portion 53 is disposed closer to the rear end side than the second reduced outer diameter portion 11 of the insulator 10, and forms the rear end (that is, the end on the rear end direction D2 side) of the metal shell 50. The crimped portion 53 is bent inward in the radial direction.

An annular space SP is formed between the inner circumferential surface of the metal shell 50 and the outer circumferential surface of the insulator 10, and is positioned on the rear end side of the metal shell 50. In the embodiment, the space SP is a space surrounded by the crimped portion 53 and the tool engagement portion 51 of the metal shell 50, and the second reduced outer diameter portion 11 and the rear end-side trunk portion 18 of the insulator 10. The first rear end-side packing 6 is disposed in the space SP on the rear end side, and the second rear end-side packing 7 is disposed in the space SP on the leading end side. In the embodiment, the rear end-side packings 6 and 7 are steel C-rings (another material may also be adopted). The gap between the rear end-side packings 6 and 7 in the space SP is filled with a powder of talc 9.

When the spark plug 100 is manufactured, the crimped portion 53 is crimped in such a way as to be bent inward. The crimped portion 53 is pressed toward the leading end direction D1 side. Accordingly, the deformed portion 58 is deformed, and the insulator 10 is pressed toward the leading end side via the packings 6 and 7 and the talc 9 in the metal shell 50. The leading end side packing 8 is pressed between the first reduced outer diameter portion 15 and the reduced inner diameter portion 56, and the gap between the metal shell 50 and the insulator 10 is sealed. Accordingly, the leaking of gas in a combustion chamber of an internal combustion engine to the outside through the gap between the metal shell 50 and the insulator 10 is suppressed. Further, the metal shell 50 is fixed to the insulator 10.

The ground electrode 30 is joined to the leading end (that is, the end on the leading end direction D1 side) of the metal shell 50. In the embodiment, the ground electrode 30 is a bar-shaped electrode. The ground electrode 30 extends toward the leading end direction D1 from the metal shell 50, is bent toward the center axis CL, and then reaches a leading end portion 31. A gap g is formed between the leading end

portion 31 and a leading end surface 20s1 (a surface of 20s1 on the leading end direction D1 side) of the center electrode 20. The ground electrode 30 is electrically conductively joined to the metal shell 50 (for example, by laser welding).

The ground electrode 30 includes a base member 35 forming the surface of the ground electrode 30, and a core portion 36 embedded in the base member 35. For example, the base member 35 is made of Inconel. The core portion 36 is made of a material (for example, pure copper) having a coefficient of thermal conductivity higher than that of the base member 35.

As described above, in the first embodiment, the magnetic substance 210 is disposed in the middle of the conductive path connecting the center electrode 20 and the terminal metal fixture 40 together. Accordingly, it is possible to suppress the occurrence of electromagnetic noise induced by discharge. Further, the conductor 220 is connected in series to at least a part of the magnetic substance 210. Accordingly, it is possible to suppress an increase in the electrical resistance between the center electrode 20 and the terminal metal fixture 40. Further, since the conductor 220 is a spiral coil, it is possible to further suppress electromagnetic noise.

#### A-2. Manufacturing Method:

A method of manufacturing the spark plug 100 in the first embodiment can be arbitrarily adopted. For example, the following manufacturing method can be adopted. First, the insulator 10, the center electrode 20, the terminal metal fixture 40, a material powder for each of the conductive sealing portions 60, 75 and 80, a material powder for the resistor 70, and the magnetic substance structure 200 are prepared. The magnetic substance structure 200 is formed by wrapping the conductor 220 around the magnetic substance 210 formed by a well-known method.

Subsequently, the center electrode 20 is inserted into the insulator 10 through an opening (hereinafter, referred to as a "rear opening 14") of the through hole 12 on the rear end direction D2 side. As illustrated in FIG. 1, the center electrode 20 is supported by the reduced inner diameter portion 16 of the insulator 10 such that the center electrode 20 is disposed at a predetermined position in the through hole 12.

Subsequently, the filling of the material powders for the first conductive sealing portion 60, the resistor 70, and the second conductive sealing portion 75 into the through hole 12 and molding of the filled powder materials are performed in the order of the members 60, 70 and 75. The filling of the powder materials into the through hole 12 is performed through the rear opening 14. The molding of the filled powder materials is performed by using a bar inserted through the rear opening 14. The material powder is molded into substantially the same shape as that of the corresponding member.

Subsequently, the magnetic substance structure 200 is inserted into the through hole 12 through the rear opening 14, and is disposed on the rear end direction D2 side of the second conductive sealing portion 75. The gap between the magnetic substance structure 200 and the inner circumferential surface 10i of the insulator 10 is filled with material powder for the covering portion 290. Subsequently, the filling of material powder for the third conductive sealing portion 80 into the through hole 12 is performed through the rear opening 14. The insulator 10 is heated up to a predetermined temperature higher than the softening point of a glass component contained in each of the material powders, and the terminal metal fixture 40 is inserted into the through hole 12 through the rear opening 14 of the through hole 12 with the insulator 10 heated at the predetermined tempera-

## 11

ture. As a result, the material powders are compressed and sintered such that the conductive sealing portions **60**, **75** and **80**, the resistor **70**, and the covering portion **290** are formed.

Subsequently, the metal shell **50** is assembled to the outer circumference of the insulator **10**, and the ground electrode **30** is fixed to the metal shell **50**. Subsequently, the ground electrode **30** is bent, and the manufacturing of a spark plug is complete.

## B. Second Embodiment

FIG. 2 is a cross-sectional view of a spark plug **100b** in a second embodiment. The spark plug **100b** is different from the spark plug **100** in the first embodiment only in that the magnetic substance structure **200** is replaced with a magnetic substance structure **200b**. The remainder of the configuration of the spark plug **100b** is the same as that of the spark plug **100** in FIG. 1. The same reference signs will be assigned to the same elements in FIG. 2 as those in FIG. 1, and description thereof will be omitted.

As illustrated, the magnetic substance structure **200b** is disposed between the resistor **70** and the terminal metal fixture **40** in the through hole **12** of the insulator **10**. On the right side of FIG. 2, a perspective view (referred to as a “first perspective view P1”) of the magnetic substance structure **200b** covered with a covering portion **290b** and a perspective view (referred to as a “second perspective view P2”) of the magnetic substance structure **200b** from which the covering portion **290b** is removed are illustrated. The second perspective view P2 illustrates a partially cut-out magnetic substance structure **200b** so as to show the internal configuration of the magnetic substance structure **200b**.

As illustrated, the magnetic substance structure **200b** includes a magnetic substance **210b** and a conductor **220b**. The conductor **220b** is cross-hatched in the second perspective view P2. The magnetic substance **210b** is a tubular member centered around the center axis **CL**. Similar to the magnetic substance **210** in FIG. 1, various magnetic materials (for example, a ferromagnetic material containing iron oxide) can be adopted as the material of the magnetic substance **210b**.

The conductor **220b** penetrates through the magnetic substance **210b** along the center axis **CL**. The conductor **220b** extends from the end of the magnetic substance **210b** on the leading end direction **D1** side to the end of the magnetic substance **210b** on the rear end direction **D2** side. Similar to the conductor **220** in FIG. 1, various conductive materials (for example, an alloy containing nickel and chromium as main components) can be adopted as the material of the conductor **220b**.

The outer circumferential surface of the magnetic substance structure **200b** is covered with the covering portion **290b**. Similar to the covering portion **290** in FIG. 1, the covering portion **290b** is a tubular member covering the magnetic substance structure **200b**. Since the covering portion **290b** is interposed between the inner circumferential surface **10i** of the insulator **10** and the outer circumferential surface of the magnetic substance structure **200b**, the positional offset between the insulator **10** and the magnetic substance structure **200b** is suppressed. Similar to the covering portion **290** in FIG. 1, various materials (glass such as borosilicate glass) can be adopted as the material of the covering portion **290b**.

A second conductive sealing portion **75b** is disposed between the magnetic substance structure **200b** and the resistor **70** in the through hole **12** while being in contact with the magnetic substance structure **200b** and the resistor **70**. A

## 12

third conductive sealing portion **80b** is disposed between the magnetic substance structure **200b** and the terminal metal fixture **40** while being in contact with the magnetic substance structure **200b** and the terminal metal fixture **40**. Similar to the conductive sealing portions **75** and **80** in FIG. 1, various conductive materials (for example, a material containing similar glass particles as those of the resistor **70**, and metal particles (Cu, Fe, and the like)) can be adopted as the material of each of the conductive sealing portions **75b** and **80b**.

The end of the magnetic substance structure **200b** on the leading end direction **D1** side, that is, the end of each of the magnetic substance structure **210b** and the conductor **220b** on the leading end direction **D1** side is electrically connected to the resistor **70** via the second conductive sealing portion **75b**. The end of the magnetic substance structure **200b** on the rear end direction **D2** side, that is, the end of each of the magnetic substance structure **210b** and the conductor **220b** on the rear end direction **D2** side is electrically connected to the terminal metal fixture **40** via the third conductive sealing portion **80b**. The first conductive sealing portion **60**, the resistor **70**, the second conductive sealing portion **75b**, the magnetic substance structure **200b**, and the third conductive sealing portion **80b** form a conductive path through which the center electrode **20** is electrically connected to the terminal metal fixture **40**. It is possible to stabilize the contact resistance between the members **20**, **60**, **70**, **75b**, **200b**, **80b** and **40** stacked on top of each other, and to stabilize the electrical resistance between the center electrode **20** and the terminal metal fixture **40** by using the conductive sealing portions **60**, **75b** and **80b**. Hereinafter, all of a plurality of members **60**, **70**, **75b**, **200b**, **290b** and **80b**, which are disposed in the through hole **12** and connect the center electrode **20** and the terminal metal fixture **40** together, may be referred to as a “connection portion **300b**”.

As described above, in the second embodiment, the magnetic substance **210b** is disposed in the middle of the conductive path connecting the center electrode **20** and the terminal metal fixture **40** together. Accordingly, it is possible to suppress the occurrence of electromagnetic noise induced by discharge. Further, the conductor **220b** is connected in series to the magnetic substance **210b**. Accordingly, it is possible to suppress an increase in the electrical resistance between the center electrode **20** and the terminal metal fixture **40**. Further, the conductor **220b** is embedded in the magnetic substance **210b**. That is, the entirety of the conductor **220b** except for both ends is covered with the magnetic substance **210b**. Accordingly, it is possible to suppress damage to the conductor **220b**. For example, the occurrence of a short circuit of the conductor **220b** induced by vibration can be suppressed.

The spark plug **100b** in the second embodiment can be manufactured using the same method as the spark plug **100** in the first embodiment. The magnetic substance structure **200b** is formed by inserting the conductor **220b** into a through hole of the magnetic substance **210b** formed by a well-known method.

## C. Reference Example

FIG. 3 is a cross-sectional view of a spark plug **100c** in a reference example. The spark plug **100c** is used as a reference example in evaluation tests to be described later. The spark plug **100c** is different from the spark plug **100** in FIG. 1 in that the magnetic substance structures **200** and the third conductive sealing portion **80** are omitted, and is different from the spark plug **100b** in FIG. 2 in that the magnetic

substance structure **200b** and the third conductive sealing portion **80b** are omitted. In the reference example, a leg portion **43c** of a terminal metal fixture **40c** is longer than the leg portion **43** in the embodiments such that the end of the leg portion **43c** on the leading end direction **D1** side reaches the vicinity of the resistor **70**. A second conductive sealing portion **75c** is disposed between the leg portion **43c** and the resistor **70** while being in contact with the leg portion **43c** and the resistor **70**. The same material as that of the second conductive sealing portion **75** in the embodiments can be adopted as the material of the second conductive sealing portion **75c**.

In FIG. 3, an intermediate position **44** (referred to as an “intermediate position **44**”) of a portion of a through hole **12c** of an insulator **10c** accommodating the leg portion **43c** is illustrated. With respect to the through hole **12c**, an inner diameter of a portion disposed on the rear end direction **D2** side of the intermediate position **44** is slightly larger than an inner diameter of a portion disposed on the leading end direction **D1** side of the intermediate position **44** (particularly, a portion accommodating the first conductive sealing portion **60**, the resistor **70**, the second conductive sealing portion **75c**, and a portion of the leg portion **43c**). However, both inner diameters may be the same.

The remainder of the configuration of the spark plug **100c** in the reference example is the same as those of the spark plugs **100** and **100b** illustrated in FIGS. 1 and 2. All of the first conductive sealing portion **60**, the resistor **70**, and the second conductive sealing portion **75c** form a connection portion **300c** connecting the center electrode **20** and the terminal metal fixture **40c** together in the through hole **12c**. The spark plug **100c** in the reference example can be manufactured using the same method as the spark plugs **100** and **100b** in the embodiments.

#### D. Evaluation Test

##### D-1. Configuration of Spark Plug Samples:

Evaluation tests performed on a plurality of types of spark plug samples will be described. Table 1 below illustrates the configuration of each sample, and each evaluation result of four evaluation tests.

TABLE 1

| No. | Configuration | Existence or Non-existence of Covering Portion | Electromagnetic Noise Characteristics | Impact Resistance Characteristics | Resistance Stability | Durability |
|-----|---------------|------------------------------------------------|---------------------------------------|-----------------------------------|----------------------|------------|
| 1   | A             | Yes                                            | 10                                    | 10                                | 10                   | 10         |
| 2   | B             | Yes                                            | 6                                     | 10                                | 10                   | 10         |
| 3   | C             | —                                              | Reference                             | 10                                | 10                   | 10         |
| 4   | D             | Yes                                            | 5                                     | 10                                | 10                   | 10         |
| 5   | E             | Yes                                            | 4                                     | 10                                | 10                   | 10         |
| 6   | A             | No                                             | 10                                    | 5                                 | 10                   | 10         |
| 7   | B             | No                                             | 6                                     | 5                                 | 10                   | 10         |
| 8   | F             | Yes                                            | 5                                     | 10                                | 10                   | 10         |
| 9   | G             | Yes                                            | 6                                     | 10                                | 10                   | 1          |
| 10  | H             | Yes                                            | 8                                     | 10                                | 10                   | 10         |
| 11  | I             | Yes                                            | —                                     | 0                                 | 0                    | 1          |
| 12  | J             | Yes                                            | —                                     | 0                                 | 0                    | 1          |
| 13  | K             | Yes                                            | 10                                    | 10                                | 10                   | 10         |

In the evaluation tests, 13 types of samples with different configurations were evaluated. The table illustrates numbers indicating sample types, reference signs indicating configuration types, the existence or non-existence of a covering portion, the evaluation results of electromagnetic noise characteristics, the evaluation results of impact resistance

characteristics, the evaluation results of resistance stability, and the evaluation results of durability.

The correlations between the reference signs indicating the configuration types and the configurations of the spark plugs are as described below.

- A: the configuration illustrated in FIG. 1
- B: the configuration illustrated in FIG. 2
- C: the configuration illustrated in FIG. 3
- D: a configuration in which the dispositions of the resistor **70** and the magnetic substance structure **200** in the configuration in FIG. 1 are switched
- E: a configuration in which the dispositions of the resistor **70** and the magnetic substance structure **200b** are switched
- F: a configuration in which the magnetic substance **210** in the configuration in FIG. 1 is replaced with a member made of alumina and having the same shape as the magnetic substance **210**
- G: a configuration in which the conductor **220b** in the configuration in FIG. 2 is replaced with a conductor with  $2\text{ k}\Omega$  resistance
- H: configuration in which the conductor **220b** in the configuration in FIG. 2 is replaced with a conductor with  $1\text{ k}\Omega$  resistance
- I: a configuration in which the third conductive sealing portion **80** is omitted from the configuration in FIG. 1
- J: a configuration in which the second conductive sealing portion **75** is omitted from the configuration in FIG. 1
- K: a configuration in which the conductor **220b** in the configuration in FIG. 2 is replaced with a conductor with  $200\Omega$  resistance

Here, as illustrated in Table 1, the existence or non-existence of the covering portions **290**, **290b** are determined independently from the configurations A to K.

Features common to the configurations A to K are as described below.

- 1) the material of the resistor **70**: a composite containing  $\text{B}_2\text{O}_3$ — $\text{SiO}_2$  based glass,  $\text{ZrO}_2$  as ceramic particles, and C as conductive material
- 2) the material of the magnetic substances **210**, **210b**: MnZn ferrite

- 3) the material of the conductors **220**, **220b**: an alloy containing nickel and chromium as main components
- 4) the material of the conductive sealing portions **60**, **75**, **75b**, **80**, **80b** and **80c**: a composite containing  $\text{B}_2\text{O}_3$ — $\text{SiO}_2$  based glass and Cu as metal particles

The electrical resistance of the conductor is the electrical resistance between the end of the conductor on the leading

end direction D1 side and the end of the conductor on the rear end direction D2 side. Hereinafter, the electrical resistance between the end of the conductor on the leading end direction D1 side and the end of the conductor on the rear end direction D2 side is referred to as an end-to-end resistance. Hereinafter, the results of each of the evaluation tests will be described.

D-2. Evaluation Test on Electromagnetic Noise Characteristics:

The electromagnetic noise characteristics were evaluated using an insertion loss measured according to the method specified in JASO D002-2. Specifically, the improvement (unit is dB) of the insertion loss at a frequency of 300 MHz when a 3<sup>rd</sup> sample was used as a datum was adopted as an evaluation result. An evaluation result denoted by "m (m is an integer which is zero or greater and ten or less)" implies that the improvement of the insertion loss with respect to the 3<sup>rd</sup> sample is m (dB) or greater and less than m+1 (dB). For example, an evaluation result denoted by "5" implies that the improvement is 5 dB or greater and less than 6 dB. An evaluation result was determined to be "10" when the improvement was 10 dB or greater. In the evaluation result, an average value of the insertion losses of five samples with the same configuration was used as the insertion loss of each type of sample. The five samples having the electrical resistance between the center electrode 20 and the terminal metal fixture 40, 40c in a range with a center value of 5 kΩ and a width of 0.6 kΩ, that is, a range of 4.7 kΩ or greater and 5.3 kΩ or less were adopted. Since 11<sup>th</sup> and 12<sup>th</sup> samples had a large variation in the electrical resistance, and five samples with the aforementioned range of electrical resistance could not be obtained, the 11<sup>th</sup> and 12<sup>th</sup> samples were not evaluated.

As illustrated in Table 1, when a 1<sup>st</sup> sample was compared to an 8<sup>th</sup> sample, the evaluation result of the 1<sup>st</sup> sample including the magnetic substance 210 was better than that of the 8<sup>th</sup> sample from which the magnetic substance 210 was omitted. As such, it was possible to suppress electromagnetic noise by providing the magnetic substance 210.

The evaluation result of each of the 1<sup>st</sup> sample and a 6<sup>th</sup> sample including the coil-shaped conductor 220 was "10" which was the highest grade, and the evaluation result of each of a 2<sup>nd</sup> sample and a 7<sup>th</sup> sample including the straight conductor 220b was "6" which is less than 10. As such, it was possible to considerably suppress electromagnetic noise by providing the coil-shaped conductor 220.

When the 1<sup>st</sup> sample was compared to a 4<sup>th</sup> sample, the evaluation result of the 1<sup>st</sup> sample in which the magnetic substance structure 200 was disposed closer to the rear end direction D2 side than the resistor 70 was better than that of the 4<sup>th</sup> sample in which the magnetic substance structure 200 was disposed closer to leading end direction D1 side than the resistor 70. Similarly, when the 2<sup>nd</sup> sample was compared to a 5<sup>th</sup> sample, the evaluation result of the 2<sup>nd</sup> sample in which the magnetic substance structure 200b was disposed closer to the rear end direction D2 side than the resistor 70 was better than that of the 5<sup>th</sup> sample in which the magnetic substance structure 200b was disposed closer to the leading end direction D1 side than the resistor 70. As such, it was possible to suppress electromagnetic noise by disposing the magnetic substance structure on the rear end direction D2 side of the resistor regardless of the configuration of the magnetic substance structure.

When at least one of the second conductive sealing portion 75 and the third conductive sealing portion 80 interposing the magnetic substance structure 200 therebetween was omitted (the 1<sup>th</sup> sample and the 12<sup>th</sup> sample), it

was difficult to stabilize the electrical resistance between the center electrode 20 and the terminal metal fixture 40. In contrast, it was possible to stabilize the electrical resistance by providing the second conductive sealing portion 75 and the third conductive sealing portion 80.

D-3. Evaluation Result of Impact Resistance Characteristics:

The impact resistance characteristics were evaluated according to the impact resistance test specified in 7.4 of JIS B8031:2006. An evaluation result denoted by "0" implies the occurrence of abnormality in the impact resistance test. When no abnormality was observed in the impact resistance test, a vibration test was additionally performed for 30 minutes. The difference between an electrical resistance measured before the evaluation test and an electrical resistance measured after the evaluation test was calculated. The electrical resistance is the electrical resistance between the center electrode 20 and the terminal metal fixture 40, 40c. An evaluation result denoted by "5" implies that an absolute value of the difference between the electrical resistances exceeds 10% of the electrical resistance before the test. An evaluation result denoted by "10" implies that an absolute value of the difference between the electrical resistances is 10% or less of the electrical resistance before the test.

As illustrated in Table 1, the evaluation result of each of the 1<sup>th</sup> sample and 12<sup>th</sup> sample, from which at least one of the second conductive sealing portion 75 and the third conductive sealing portion 80 interposing the magnetic substance structure 200 therebetween was omitted, was "0". In contrast, the evaluation results of the 1<sup>st</sup> to 10<sup>th</sup> samples and a 13<sup>th</sup> sample, which include two conductive sealing portions (for example, the conductive sealing portions 75 and 80 in FIG. 1) interposing the magnetic substance structure 200, 200b therebetween, were "5" or "10" which was better than those of the 1<sup>th</sup> sample and the 12<sup>th</sup> sample. As such, by interposing the magnetic substance structure 200, 200b between the two conductive sealing portions, it was possible to improve impact resistance.

Further, the evaluation result of each of the 6<sup>th</sup> sample and 7<sup>th</sup> sample, in which the magnetic substance structure 200, 200b was interposed between the two conductive sealing portions but which did not include the covering portion 290, 290b, the evaluation result of each of these samples was "5". In contrast, the evaluation result of each of the 1<sup>st</sup> to 5<sup>th</sup> samples, the 8<sup>th</sup> to 10<sup>th</sup> samples, and the 13<sup>th</sup> sample, which include the two conductive sealing portions interposing the magnetic substance structure 200, 200b therebetween and the covering portion 290, 290b, was "10". As such, it was possible to considerably improve the impact resistance by providing the covering portion 290, 290b. However, the covering portion 290, 290b may be omitted.

D-4. Evaluation Result of Resistance Stability:

The resistance stability was evaluated based on a standard deviation in the electrical resistances between the center electrode 20 and the terminal metal fixture 40, 40c. As described above, the spark plugs used in the evaluation tests were manufactured by heating the insulator 10 in a state where the material of the connection portion (for example, the connection portion 300 in FIG. 1) was disposed in the through hole 12, 12c. The powder materials of the conductive sealing portions 60, 75, 75b, 75c, 80, and 80b might flow due to the heating. A variation in the electrical resistance might occur due to the flowing of the powder materials. The magnitude in the variation was evaluated. Specifically, 100 spark plugs with the same configuration were manufactured for each sample type. The electrical resistances between the center electrode 20 and the terminal metal fixture 40, 40c were measured, and a standard devia-

tion in the measured electrical resistances was calculated. An evaluation result denoted by "0" implies that the standard deviation is greater than 0.8, an evaluation result denoted by "5" implies that the standard deviation is greater than 0.5 and 0.8 or less, and an evaluation result denoted by "10" implies that the standard deviation is 0.5 or less.

As illustrated in Table 1, the evaluation result of each of the 1<sup>th</sup> sample and the 12<sup>th</sup> sample, from which at least one of the second conductive sealing portion 75 and the third conductive sealing portion 80 interposing the magnetic substance structure 200 therebetween was omitted, was "0". In contrast, the evaluation result of each of the 1<sup>st</sup> to 10<sup>th</sup> samples, and the 13<sup>th</sup> sample, which include the two conductive sealing portions (for example, the conductive sealing portions 75 and 80 in FIG. 1) interposing the magnetic substance structures 200, 200b therebetween, was "10" which was better than those of the 1<sup>th</sup> sample and the 12<sup>th</sup> sample. As such, by interposing the magnetic substance structure 200, 200b between the two conductive sealing portions, it was possible to considerably stabilize the electrical resistance.

#### D-5. Evaluation Result of Durability:

The durability is durability against discharge. The spark plug sample was connected to an automotive transistorized ignition system, and discharge was repeatedly performed under the following conditions so as to evaluate the durability.

Temperature: 350 degrees Celsius

Voltage Applied to Spark Plug: 20 kV

Discharge Period: 3,600 incidences/minute

Operation Time: 100 hours

The evaluation test was performed under the aforementioned conditions, and thereafter, the electrical resistance between the center electrode 20 and the terminal metal fixture 40, 40c was measured at a room temperature. The evaluation result was determined to be "10" when the electrical resistance after the evaluation test was less than 1.5 times the electrical resistance before the evaluation test. The evaluation result was determined to be "1" when the electrical resistance after the evaluation test was greater than or equal to 1.5 times the electrical resistance before the evaluation test.

As illustrated in Table 1, the evaluation result of the 2<sup>nd</sup> sample including the conductor 220b was "10". The evaluation result of the 13<sup>th</sup> sample including the conductor with 200Ω resistance instead of the conductor 220b was "10". The evaluation result of the 10<sup>th</sup> sample including the conductor with 1 kΩ resistance instead of the conductor 220b was "10". The evaluation result of the 9<sup>th</sup> sample including the conductor with 2 kΩ resistance instead of the conductor 220b was "1". The end-to-end resistance of the conductor 220b was approximately 50Ω. As such, it was possible to improve durability against discharge by reducing the end-to-end resistance of the conductor (specifically, the conductor connected to the magnetic substance 210b) of the magnetic substance structure.

The reason it was possible to improve durability against discharge by reducing the end-to-end resistance of the conductor of the magnetic substance structure can be estimated as follows. That is, since current flows through the conductor connected to the magnetic substance 210b during discharge, the conductor generates heat. The magnitude of current during discharge is adjusted in such a way that a proper spark occurs at the gap g regardless of the internal configuration of the spark plug. Accordingly, the greater the end-to-end resistance of the conductor is, the higher the temperature of the conductor may become. When the tem-

perature of the conductor is increased, a short circuit of the conductor is more likely to occur. When the conductor is short circuited, the electrical resistance between the center electrode 20 and the terminal metal fixture 40 may be increased. In addition, when the temperature of the conductor is increased, the temperature of the magnetic substance 210b is also increased. The magnetic substance 210b is prone to damage when the temperature of the magnetic substance 210b is high compared to when the temperature is low (for example, the cracking of the magnetic substance 210b occurs). An increase in the end-to-end resistance of the magnetic substance 210b induced by damage to the magnetic substance 210b may cause an increase in the electrical resistance between the center electrode 20 and the terminal metal fixture 40. As described above, the smaller the end-to-end resistance of the conductor is, the further it is possible to suppress the occurrence of damage to the magnetic substance 210b and a short circuit of the conductor. As a result, it can be estimated that it is possible to improve durability against discharge. Further, when the end-to-end resistance of the conductor is high, since current flows along the surface of the conductor during discharge, electromagnetic noise may occur. For this reason, the conductor of the magnetic substance structure preferably has a low end-to-end resistance.

The end-to-end resistances of the conductors 220b of the 2<sup>nd</sup>, the 13<sup>th</sup>, and 10<sup>th</sup> samples, the evaluation results of which were "10" indicating good durability, were 50Ω, 200Ω, and 1 kΩ, respectively. An arbitrary value among these values can be adopted as the upper limit of a preferable range (range of a lower limit or greater and an upper limit or less) of the end-to-end resistance of the conductor 220b. An arbitrary value less than or equal to the upper limit among these values can be adopted as the lower limit. For example, a value of 1 kΩ or less can be adopted as the end-to-end resistance of the conductor 220b. More preferably, a value of 200Ω or less can be adopted as the end-to-end resistance of the conductor 220b. In addition to the aforementioned values, a value of 0Ω can be adopted as the lower limit of the preferable range of the end-to-end resistance of the conductor 220b.

The aforementioned description has been given with reference to the evaluation results of the 2<sup>nd</sup>, the 10<sup>th</sup>, the 9<sup>th</sup>, and the 13<sup>th</sup> samples with the configuration illustrated in FIG. 2. However, it can be estimated that the relationship between heat generation of the conductor and the likeliness of occurrence of a failure (a short circuit of the conductor or damage to the magnet) can be applied regardless of the configuration of the magnetic substance structure. Accordingly, also in the spark plug with the configuration illustrated in FIG. 1, it can be estimated that, the lower the end-to-end resistance of the coil-shaped conductor 220 is, the further it is possible to suppress the occurrence of a short circuit of the conductor 220 or damage to the magnetic substance 210 to thus improve durability against discharge. Conductive metal such as an iron material or copper is preferably adopted as the material of the coil-shaped conductor 220. Particularly, stainless steel or a nickel alloy is preferably adopted upon consideration of heat resistance and costs.

During discharge, current may flow through not only the conductor 220, 220b but also the magnetic substance 210, 210b. Accordingly, the magnetic substance structure 200, 200b which is an assembly of the magnetic substance 210, 210b and the conductor 220, 200b preferably has low end-to-end resistances so as to suppress the occurrence of damage to the magnetic substance 210, 210b. For example, a range of 0Ω or greater and 3 kΩ or less can be adopted as

a preferable range of the end-to-end resistance of the magnetic substance structure **200**, **200b**. However, a value greater than 3 kΩ may be adopted. The end-to-end resistances of the conductors of the 2<sup>nd</sup>, the 13<sup>th</sup>, and 10<sup>th</sup> samples, the evaluation results of which showed good durability, were 50Ω, 200Ω, and 1 kΩ, respectively. When it is taken into consideration that such conductors are adopted, an arbitrary value among these end-to-end resistances can be adopted as the upper limit of the preferable range (range of a lower limit or greater and an upper limit or less) of the end-to-end resistance of the magnetic substance structure **200**, **200b**. An arbitrary value less than or equal to the upper limit among these values can be adopted as the lower limit. For example, a value of 1 kΩ or less can be adopted as the end-to-end resistance of the magnetic substance structure **200**, **200b**. More preferably, a value of 200Ω or less can be adopted as the end-to-end resistance of the magnetic substance structure **200**, **200b**. In addition to the aforementioned values, a value of 0Ω can be adopted as the lower limit of the preferable range of the end-to-end resistance of the magnetic substance structure **200**, **200b**.

Preferably, the end-to-end resistance of the conductor **220**, **220b** is respectively lower than that of the magnetic substance **210**, **210b** so as to suppress heat generation of the magnetic substance structure **200**, **200b**. In this configuration, it is possible to reduce the end-to-end resistance of the magnetic substance structure **200**, **200b** by connecting the conductor **220**, **220b** to the magnetic substance **210**, **210b**. As a result, it is possible to suppress heat generation of the magnetic substance structure **200**, **200b**. In each of the 1<sup>st</sup> to the 13<sup>th</sup> samples, the end-to-end resistance of the magnetic substance **210**, **210b** was several kΩ and was greater than the end-to-end resistance of the conductor (for example, the conductor **220**, **220b**). As illustrated in Table 1, the evaluation results of the 1<sup>st</sup> to 8<sup>th</sup>, the 10<sup>th</sup>, and the 13<sup>th</sup> samples showed good durability.

As illustrated in Table 1, the evaluation results of the 11<sup>th</sup> and the 12<sup>th</sup> samples, in which at least one of the second conductive sealing portion **75** and the third conductive sealing portion **80** interposing the magnetic substance structure **200** therebetween was omitted, were “1”. Each of the 1<sup>st</sup> to 8<sup>th</sup>, the 10<sup>th</sup>, and the 13<sup>th</sup> samples with a good evaluation result of “10” included two conductive sealing portions (for example, the conductive sealing portions **75** and **80** in FIG. 1) between which the magnetic substance structure **200**, **200b** was interposed. As such, since the magnetic substance structure **200**, **200b** was interposed between the two conductive sealing portions, it was possible to improve durability against discharge.

The following method can be adopted as a method of measuring the end-to-end resistance of the magnetic substance structure of the spark plug. Hereinafter, the spark plugs **100** and **100b** in FIGS. 1 and 2 will be described as examples. First, an operator disassembles the metal shell **50** from the insulator **10**, cuts the insulator **10** using a cutting tool such as a diamond blade, and takes the connection portion **300**, **300b** disposed in the through hole **12** out of the through hole **12**. Subsequently, the operator respectively disassembles the conductive sealing portions in contact with the magnetic substance structure **200**, **200b** from the magnetic substance structure **200**, **200b** using a cutting tool such as a nippers. Subsequently, after the operator observes the internal structure of each of the covering portion **290**, **290b** in contact with the magnetic substance structure **200**, **200b** using a CT scanner, the operator disassembles the covering portion **290**, **290b** from the magnetic substance structure **200**, **200b** by cutting and grinding the magnetic substance

structure **200**, **200b**. The operator brings the probes of a resistance meter into contact with both ends (on the leading end direction **D1** side and the rear end direction **D2** side) of the magnetic substance structure **200**, **200b** obtained in this manner, and measures an end-to-end resistance therebetween.

The following method can be adopted as a method of measuring the end-to-end resistance of the conductor of the magnetic substance structure. That is, the operator acquires the conductor **220**, **220b** by removing the magnetic substance **210**, **210b** from the magnetic substance structure **200**, **200b** obtained by the aforementioned method using a cutting tool such as nippers. The operator brings the probes of a resistance meter into contact with both ends on the leading end direction **D1** side and the rear end direction **D2** side of the conductor **220**, **220b** obtained in this manner, and measures an end-to-end resistance therebetween.

The following method can be adopted as a method of measuring the end-to-end resistance of the magnetic substance of the magnetic substance structure. That is, after the operator observes the internal structure of the magnetic substance structure **200**, **200b** using a CT scanner, the operator obtains the magnetic substance **210**, **210b** by cutting and grinding the magnetic substance structure **200**, **200b**. The operator brings the probes of a resistance meter into contact with both ends on the leading end direction **D1** side and the rear end direction **D2** side of the magnetic substance **210**, **210b**, and measures an end-to-end resistance therebetween.

At least one of both ends on the leading end direction **D1** side and the rear end direction **D2** side of each of the magnetic substance structure, the conductor, and the magnetic substance may be a surface. In this case, the minimum end-to-end resistance obtained by bringing the probe of a resistance meter into contact with the surface at an arbitrary position is adopted.

#### E. Third Embodiment

##### E-1. Configuration of Spark Plug:

FIG. 4 is a cross-sectional view of a spark plug **100d** in a third embodiment. In the third embodiment, a magnetic substance structure **200d** is provided instead of the magnetic substance structures **200** and **200b** in FIGS. 1 and 2. A perspective view of the magnetic substance structure **200d** is illustrated on the right side of FIG. 4. The magnetic substance structure **200d** is a tubular member centered around the center axis **CL**. A portion of the center electrode **20** on the rear end direction **D2** side, a first conductive sealing portion **60d**, a resistor **70d**, a second conductive sealing portion **75d**, the magnetic substance structure **200d**, a third conductive sealing portion **80d**, and a leg portion **43d** of a terminal metal fixture **40d** are disposed in a through hole **12d** of an insulator **10d** sequentially from the leading end direction **D1** side toward the rear end direction **D2** side. The magnetic substance structure **200d** is disposed on the rear end direction **D2** side of the resistor **70d**. All of the members **60d**, **70d**, **75d**, **200d** and **80d** form a connection portion **300d** connecting the center electrode **20** and the terminal metal fixture **40d** together in the through hole **12d**. The remainder of the configuration of the spark plug **100d** in the third embodiment is substantially the same as the configuration of each of the spark plugs **100** and **100b** in FIGS. 1 and 2. In FIG. 4, the same reference signs will be assigned to portions of the spark plug **100d** in the third embodiment, which

correspond to the portions of each of the spark plugs 100 and 100b in FIGS. 1 and 2. The description thereof will be omitted.

FIG. 5 shows views illustrating the magnetic substance structure 200d. A perspective view of the magnetic substance structure 200d is illustrated on the left upper side of FIG. 5. The perspective view illustrates the partially cut-out magnetic substance structure 200d. A cross-section 900 in the perspective view is the planar cross-section of the magnetic substance structure 200d, which includes the center axis CL. An enlarged schematic view of a portion 800 (hereinafter, referred to as a "target region 800") of the cross-section 900 is illustrated on the center upper side of FIG. 5. The target region 800 is a rectangular region having the center axis CL as the center line, and is formed by two sides parallel with the center axis CL and two sides perpendicular to the center axis CL. The shape of the target region 800 is symmetric with respect to the center axis CL serving as the symmetric axis, that is, the target region 800 has a line-symmetric shape. A first length La in FIG. 5 is a length in a direction perpendicular to the center axis CL of the target region 800, and a second length Lb is a length parallel with the center axis CL of the target region 800. The first length La is 2.5 mm, and the second length Lb is 5.0 mm.

As illustrated, the target region 800 (that is, the cross-section of the magnetic substance structure 200d) contains a ceramic region 810, a conductive region 820, and a magnetic region 830. The magnetic region 830 is formed by a plurality of grain-shaped regions 835 (hereinafter, referred to as "magnetic grain regions 835" or also simply referred to as "grain regions 835"). The magnetic region 830 is formed of an iron-containing oxide as a magnetic substance. A spinel ferrite ((Ni, Zn)Fe<sub>2</sub>O<sub>4</sub>), a hexagonal ferrite (BaFe<sub>12</sub>O<sub>19</sub>), or the like can be adopted as the iron-containing oxide. The plurality of magnetic grain regions 835 are formed of iron-containing oxide power as the material of the magnetic substance structure 200d. For example, one magnetic grain region 835 can be formed of one of iron-containing oxide grains contained in the material powder. A plurality of iron-containing oxide grains contained in the material powder are stuck together to form one grain-shaped structure. The magnetic grain region 835 can be formed by the one grain-shaped structure which has been formed. The grain-shaped structure is formed by adding a binder into a material powder of an iron-containing oxide, and mixing the binder and the material powder together. A plurality of iron-containing oxide grains are stuck together by the binder, thereby resulting in formation of a grain-shaped structure having a large diameter. Hereinafter, when it is not necessary to distinguish between one grain and one grain-shaped structure formed by a plurality of grains, a three-dimensional grain-shaped element forming one magnetic grain region 835 is referred to as a "magnetic grain". One magnetic grain region 835 illustrates the cross-section of one magnetic grain.

The surface of each of a plurality of magnetic grains forming the plurality of magnetic grain-shaped regions 835 is covered with a covering layer made of a conductive substance, which is not illustrated. Metal (Ni, Cu, and the like), perovskite type oxides (SrTiO<sub>3</sub>, SrCrO<sub>3</sub>, and the like), carbon (C), carbon compounds (Cr<sub>3</sub>C<sub>2</sub>, TiC, and the like), or the like can be adopted as the conductive substance.

The conductive region 820 in FIG. 5 illustrates the cross-section of the covering layer which is made of a conductive substance and formed on the surface of the magnetic grain. As illustrated, the edge of the magnetic grain region 835 is covered with the conductive region 820. The

conductive region 820 is formed of a plurality of covering regions 825 with which the plurality of magnetic grain regions 835 are respectively covered. The region covering one magnetic grain region 835 corresponds to one covering region 825. A grain-shaped region 840 (referred to as a "composite grain region 840") is formed by one magnetic grain region 835 and one covering region 825 covering the one magnetic grain region 835. As illustrated, a plurality of composite grain regions 840 are disposed in such a way that the covering regions 825 are in contact with each other. The plurality of covering regions 825 in contact with each other form a current path extending from the rear end direction D2 side toward the leading end direction D1 side.

Two composite grain regions 840 may be disposed separately from each other in the target region 800 (that is, the cross-section 900), which is not illustrated. The two composite grain regions 840 positioned away from each other in the target region 800 may illustrate the cross-sections of two three-dimensional grain-shaped regions which are in contact with each other at a position at a front side or a back side of the target region 800. As such, the plurality of composite grain regions 840 in contact with each other or positioned away from each other in the target region 800 are capable of forming a current path extending from the rear end direction D2 side toward the leading end direction D1 side. During discharge, current flows through the plurality of covering regions 825 (that is, the conductive region 820) of the plurality of composite grain regions 840 in the magnetic substance structure 200d.

As described above, the magnetic region 830 is covered with the conductive region 820. That is, the current path is formed to surround the magnetic substance. When the magnetic substance is disposed in the vicinity of the conductive path, electromagnetic noise induced by discharge is suppressed. For example, the conductive path serves as an inductance element, and suppresses electromagnetic noise. In addition, an increase in the impedance of the conductive path suppresses electromagnetic noise.

The ceramic region 810 is formed of a ceramic. For example, a ceramic containing at least one of silicon (Si), boron (B), and phosphorous (P) can be adopted as the ceramic. For example, a ceramic such as glass described in the first embodiment can be adopted. For example, a substance containing one or more oxides arbitrarily selected from silica (SiO<sub>2</sub>), boric acid (B<sub>2</sub>O<sub>5</sub>), and phosphoric acid (P<sub>2</sub>O<sub>5</sub>) can be adopted as the glass. As illustrated, the plurality of composite grain regions 840 (that is, the plurality of magnetic grain regions 835 and the plurality of covering regions 825 covering the plurality of magnetic grain regions 835) are surrounded by the ceramic region 810.

One grain region 835 and one circle 835c are illustrated on the center lower side of FIG. 5. The circle 835c is an imaginary circle (hereinafter, referred to as an "imaginary circle 835c") having the same area as that of the grain region 835. A diameter Dc in the drawing is the diameter of the imaginary circle 835c. The diameter Dc is a diameter (hereinafter, referred to as an "approximate diameter Dc") obtained by the approximation of the grain region 835 to a circle. As the area of the grain region 835 increases, the approximate diameter Dc also increases.

The fact that the approximate diameter Dc of each of the plurality of grain regions 835 is large implies that the area of each of the plurality of covering regions 825 is large, that is, the current path is large. The durability of the current path is improved as the current path is larger. Accordingly, it is possible to further improve the durability of the current path, that is, the durability of the magnetic substance structure

200d as a number of magnetic grain regions 835 with a large approximate diameter Dc (for example, the approximate diameter Dc in a range of 400  $\mu\text{m}$  or greater and 1,500  $\mu\text{m}$  or less) among the plurality of grain regions 835 contained in the target region 800 is increased.

A partially enlarged view of the target region 800 is illustrated on the right lower side of FIG. 5. A minimum thickness T in the drawing is the minimum thickness of the conductive region 820 in the target region 800. When the minimum thickness T is small, the durability of the conductive region 820 may be reduced. When the minimum thickness T is large, a large amount of the material of the conductive region 820 is required to form the magnetic substance structure 200d.

The ceramic region 810 is formed of a ceramic powder as the material of the magnetic substance structure 200d. Accordingly, pores may be formed in the ceramic region 810 in the target region 800. An enlarged view of the ceramic region 810 is illustrated on the left lower side of FIG. 5. As illustrated, pores 812 are formed in the ceramic region 810. During discharge of the spark plug 100d, partial discharge may also occur in the pores 812. The partial discharge occurring in the pores 812 may cause aging of the magnetic substance structure 200d, and the occurrence of electromagnetic noise. Accordingly, a proportion of the pores 812 in the magnetic substance structure 200d (a proportion of an area of the pores 812 to an area of the remainder of the target region 800 which is other than the magnetic regions 830) is preferably small.

FIG. 6 is a partial enlarged view of the cross-sectional view in FIG. 4. FIG. 6 illustrates the vicinity of the crimped portion 53 of the metal shell 50. A protrusion distance Ld in FIG. 6 is the distance between a rear end 53e of the crimped portion 53 (that is, the rear end of the metal shell 50) and a rear end 200d e of the magnetic substance structure 200d, and is parallel to the center axis CL. When the rear end 200d e of the magnetic substance structure 200d is positioned closer to the rear end direction D2 side than the rear end 53e of the metal shell 50, the protrusion distance Ld is a positive value. Further, as the protrusion distance Ld increases, the distance between the leg portion 43d of the terminal metal fixture 40d and the metal shell 50 also increases.

As illustrated, the insulator 10d is disposed between the terminal metal fixture 40d and the metal shell 50. That is, the terminal metal fixture 40d and the metal shell 50 serve as a capacitor with the insulator 10d interposed between the terminal metal fixture 40d and the metal shell 50. Accordingly, electromagnetic noise may flow from the terminal metal fixture 40d to the metal shell 50 having the same potential as that of the ground electrode 30 via the insulator 10d. As a result, the suppression effects of electromagnetic noise may be reduced. Here, when the protrusion distance Ld is large, the distance between the terminal metal fixture 40d and the metal shell 50 is increased, thereby resulting in a reduction in the capacitance of the capacitor. When the capacitor has a low capacitance, the magnitude (absolute value) of the impedance of the capacitor is large. Accordingly, it is possible to suppress electromagnetic noise compared to when the distance between the terminal metal fixture 40d and the metal shell 50 is short.

#### E-2. Manufacturing Method:

The spark plug 100d including the magnetic substance structure 200d can be manufactured according to the same sequence as in the manufacturing method described in the first embodiment. The members in the through hole 12d of the insulator 10d are formed as described below. Material powders for the conductive sealing portions 60d, 75d and

80d, the resistor 70d, and the magnetic substance structure 200d are prepared. The same material powders as for the conductive sealing portions 60, 75 and 80, and the resistor 70 in the first embodiment can be adopted as the material powders for the conductive sealing portions 60d, 75d and 80d, and the resistor 70d. For example, the material powder for the magnetic substance structure 200d is prepared as described below. A covering layer, which is made of a conductive substance and covers the surface of a magnetic substance particle, is formed by applying non-electrolytic plating to the magnetic substance powder. The material powder for the magnetic substance structure 200d is prepared by mixing the magnetic powder covered with the covering layer and a ceramic powder together. The covering layer may be formed by coating the surface of the magnetic powder with a binder instead of plating, and joining conductive substance particles to the surfaces of the magnetic substance particles. The material powder for the magnetic substance structure 200d may be prepared by mixing the magnetic powder covered with the covering layers and a ceramic powder together.

Subsequently, similar to the manufacturing method in the first embodiment, the center electrode 20 is disposed at a predetermined position in which the center electrode 20 is supported by the reduced inner diameter portion 16 in the through hole 12d. The filling of the material powders for the first conductive sealing portion 60d, the resistor 70d, the second conductive sealing portion 75d, the magnetic substance structure 200d, and the third conductive sealing portion 80d into the through hole 12d, and molding of the filled powder materials are performed in the order of the members 60d, 70d, 75d, 200d and 80d. The filling of the powder materials into the through hole 12d is performed through the rear opening 14. The molding of the filled powder materials is performed by using a bar inserted through the rear opening 14. The material powder is molded into substantially the same shape as that of the corresponding member.

The insulator 10d is heated up to a predetermined temperature higher than the softening point of a glass component contained in each of the material powders, and the terminal metal fixture 40d is inserted into the through hole 12d through the rear opening 14 of the through hole 12d with the insulator 10d heated at the predetermined temperature. As a result, the material powders are compressed and sintered such that the conductive sealing portions 60d, 75d and 80d, the resistor 70d, and the magnetic substance structure 200d are formed.

#### F. Fourth Embodiment

FIG. 7 is a cross-sectional view of a spark plug 100e in a fourth embodiment. The spark plug 100e is different from the spark plug 100d in FIG. 4 in that the resistor 70d and the second conductive sealing portion 75d are omitted. In the spark plug 100e according to the fourth embodiment, the center electrode 20 is connected to the magnetic substance structure 200d via a first conductive sealing portion 60e, and the magnetic substance structure 200d is connected to a leg portion 43e of a terminal metal fixture 40e via a second conductive sealing portion 80e. All of the members 60e, 200d and 80e form a connection portion 300e connecting the center electrode 20 and the terminal metal fixture 40e together in the through hole 12d. In FIG. 7, the entirety of the magnetic substance structure 200d is disposed closer to the leading end direction D1 side than the rear end 53e of the metal shell 50. However, at least a part of the magnetic

substance structure **200d** may be disposed closer to the rear end direction D2 side than the rear end **53e** of the metal shell **50**. The remainder of the configuration of the spark plug **100e** in the fourth embodiment is substantially the same as in the spark plug **100d** illustrated in FIG. 4. In FIG. 7, the same reference signs will be assigned to portions of the spark plug **100e** in the fourth embodiment, which correspond to the portions of the spark plug **100d** in FIG. 4. The description thereof will be omitted.

The magnetic substance structure **200d** in the fourth embodiment is the same as the magnetic substance structure **200d** illustrated in FIG. 4. As described above, since the conductive region **820** forming a current path is positioned in the vicinity of the magnetic region **830** in the magnetic substance structure **200d**, the magnetic substance structure **200d** is capable of suppressing electromagnetic noise.

The spark plug **100e** in the fourth embodiment can be manufactured according to a similar manufacturing method as for the spark plug **100d** illustrated in FIG. 4. The same material powders for the conductive sealing portions **60d** and **80d** in FIG. 4 can be adopted as material powders for the conductive sealing portions **60e** and **80e**.

#### G. Evaluation Test

##### 10 G-1. Outline

Evaluation tests performed on a plurality of types of samples of the spark plug **100d** in FIG. 4 and a plurality of types of samples of the spark plug **100e** in FIG. 7 will be described. Tables 2, 3, and 4 below illustrate the configuration and the evaluation test result of each sample.

TABLE 2

| Fe-containing Oxide |                                                     |              |                                |              |                               |              |                    |                      |
|---------------------|-----------------------------------------------------|--------------|--------------------------------|--------------|-------------------------------|--------------|--------------------|----------------------|
| No.                 | Composition                                         | Grain Number | Conductive Substance Ceramic   |              |                               | Porosity (%) | Protrusion Ld (mm) | Sealing Portion 75 d |
|                     |                                                     |              | 400 to 1,500 ( $\mu\text{m}$ ) | Coverage (%) | Thickness T ( $\mu\text{m}$ ) |              |                    |                      |
| A-1                 | $\text{Fe}_2\text{O}_3$                             | 4            | 50                             | 0.5          | Si, Mg, Ba, Ca                | 5            | —                  | N                    |
| A-2                 | $\text{Fe}_3\text{O}_4$                             | 5            | 55                             | 0.8          | P, Mg, Ba, Na                 | 4.8          | —                  | N                    |
| A-3                 | (Ni, Zn) $\text{Fe}_2\text{O}_4$                    | 3            | 69                             | 0.5          | B, Ca, Mg, P, Na, K           | 4.6          | —                  | N                    |
| A-4                 | FeO                                                 | 5            | 72                             | 28           | Si, P, Mg, Ba, Li             | 4.3          | —                  | N                    |
| A-5                 | $\text{BaFe}_{12}\text{O}_{19}$                     | 4            | 100                            | 30           | B, Ca, Mg, P, Na, K           | 4.6          | —                  | N                    |
| A-6                 | $\text{SrFe}_{12}\text{O}_{19}$                     | 4            | 94                             | 31           | Si, B, Mg, Sr                 | 4.3          | —                  | N                    |
| A-7                 | $\text{Y}_3\text{Fe}_5\text{O}_{12}$                | 6            | 56                             | 0.6          | P, Mg, Ba, Na                 | 4.3          | —                  | N                    |
| A-8                 | $\text{Ba}_2\text{Mg}_2\text{Fe}_{12}\text{O}_{22}$ | 7            | 63                             | 0.8          | B, Ca, Mg, Li                 | 4.2          | —                  | N                    |
| A-9                 | (Ni, Zn) $\text{Fe}_2\text{O}_4$                    | 7            | 69                             | 26           | Si, P, Mg, Ba, Li             | 4            | —                  | N                    |
| A-10                | $\text{NiFe}_2\text{O}_4$                           | 8            | 74                             | 28           | B, Ca, Mg, P, Na, K           | 4.1          | —                  | N                    |
| A-11                | $\text{Fe}_2\text{O}_3$                             | 7            | 63                             | 29           | P, Mg, Ca, Ti, K, Li          | 4            | —                  | N                    |

  

| Resistor No. | 70 d | Noise (dB) Before Durability Test |           |           | Noise (dB) After Noise Test |           |           |
|--------------|------|-----------------------------------|-----------|-----------|-----------------------------|-----------|-----------|
|              |      | 30 (MHz)                          | 100 (MHz) | 200 (MHz) | 30 (MHz)                    | 100 (MHz) | 200 (MHz) |
| A-1          | N    | 65                                | 60        | 56        | 76                          | 70        | 64        |
| A-2          | N    | 64                                | 58        | 55        | 76                          | 71        | 65        |
| A-3          | N    | 64                                | 59        | 54        | 77                          | 70        | 63        |
| A-4          | N    | 66                                | 58        | 54        | 76                          | 70        | 64        |
| A-5          | N    | 65                                | 61        | 55        | 74                          | 71        | 65        |
| A-6          | N    | 66                                | 59        | 54        | 76                          | 71        | 64        |
| A-7          | N    | 59                                | 54        | 49        | 67                          | 62        | 57        |
| A-8          | N    | 60                                | 55        | 50        | 68                          | 63        | 58        |
| A-9          | N    | 59                                | 55        | 48        | 67                          | 63        | 56        |
| A-10         | N    | 58                                | 54        | 49        | 66                          | 62        | 57        |
| A-11         | N    | 60                                | 54        | 50        | 68                          | 62        | 58        |

TABLE 3

| Fe-containing Oxide |                                                     |                                                   |                      |                                  |                                  |                 |                                   |                            |
|---------------------|-----------------------------------------------------|---------------------------------------------------|----------------------|----------------------------------|----------------------------------|-----------------|-----------------------------------|----------------------------|
| No.                 | Composition                                         | Grain Number<br>400 to<br>1,500 ( $\mu\text{m}$ ) | Conductive Substance |                                  | Ceramic<br>Elements<br>Contained | Porosity<br>(%) | Protrusion<br>Distance<br>Ld (mm) | Sealing<br>Portion<br>75 d |
|                     |                                                     |                                                   | Coverage<br>(%)      | Thickness<br>T ( $\mu\text{m}$ ) |                                  |                 |                                   |                            |
| A-12                | $\text{NiFe}_2\text{O}_4$                           | 9                                                 | 58                   | 1                                | P, Si, K, Li                     | 4               | —                                 | N                          |
| A-13                | $(\text{Ni}, \text{Zn})\text{Fe}_2\text{O}_4$       | 8                                                 | 62                   | 25                               | B, Ca, Mg, Li                    | 3.8             | —                                 | N                          |
| A-14                | $\text{NiFe}_2\text{O}_4$                           | 9                                                 | 66                   | 11                               | B, Ca, Mg,<br>P, Na, K           | 3.9             | —                                 | N                          |
| A-15                | $\text{Fe}_2\text{O}_3$                             | 6                                                 | 69                   | 16                               | Si, P, Mg,<br>Ba, Li             | 3.8             | —                                 | N                          |
| A-16                | $\text{Y}_3\text{Fe}_5\text{O}_{12}$                | 7                                                 | 61                   | 19                               | B, Ca, Mg,<br>P, Na, K           | 3.7             | —                                 | N                          |
| A-17                | $(\text{Mn}, \text{Zn})\text{Fe}_2\text{O}_4$       | 7                                                 | 58                   | 22                               | B, Ca, Mg,<br>P, Na, K           | 3.6             | —                                 | N                          |
| A-18                | $\text{Ba}_2\text{Co}_2\text{Fe}_{12}\text{O}_{22}$ | 9                                                 | 78                   | 13                               | P, Mg, Ca,<br>Ti, K, Li          | 3.5             | 10                                | A                          |
| A-19                | $\text{Fe}_2\text{O}_3$                             | 10                                                | 69                   | 12                               | Si, Mg, Ba,<br>Ca, Na            | 3.3             | 10                                | A                          |
| A-20                | $\text{Fe}_3\text{O}_4$                             | 9                                                 | 93                   | 10                               | P, Mg, Ba,<br>Na                 | 3.8             | 10                                | A                          |
| A-21                | $(\text{Ni}, \text{Zn})\text{Fe}_2\text{O}_4$       | 11                                                | 95                   | 8                                | B, Ca, Mg,<br>P, Na, K           | 3.8             | 10                                | A                          |
| A-22                | $\text{CuFe}_2\text{O}_4$                           | 10                                                | 88                   | 5                                | Si, P, Mg,<br>Ba, Li             | 3.6             | 10                                | A                          |
| A-23                | $(\text{Ni}, \text{Zn})\text{Fe}_2\text{O}_4$       | 9                                                 | 81                   | 4                                | B, Ca, Mg,<br>P, Na, K           | 3.9             | 10                                | A                          |
| A-24                | $(\text{Mn}, \text{Zn})\text{Fe}_2\text{O}_4$       | 9                                                 | 77                   | 3                                | B, Ca, Mg,<br>P, Na, K           | 3.8             | 1                                 | A                          |
| A-25                | $\text{Ba}_2\text{Co}_2\text{Fe}_{12}\text{O}_{22}$ | 11                                                | 92                   | 6                                | B, Ca, Mg,<br>P, Na, K           | 3.7             | 3                                 | A                          |
| A-26                | $(\text{Ni}, \text{Zn})\text{Fe}_2\text{O}_4$       | 10                                                | 69                   | 5                                | P, Mg, Ca,<br>Ti, K, Li          | 3.8             | 5                                 | A                          |
| A-27                | $\text{CuFe}_2\text{O}_4$                           | 9                                                 | 78                   | 4                                | P, Si, K,<br>Li                  | 3.8             | 7                                 | A                          |
| A-28                | $\text{BaFe}_{12}\text{O}_{19}$                     | 8                                                 | 83                   | 7                                | B, Ca, Mg,<br>Li                 | 3.6             | 9                                 | A                          |
| A-29                | $\text{Fe}_2\text{O}_3$                             | 6                                                 | 56                   | 30                               | Si, P, Mg,<br>Ba, Li             | 6.6             | —                                 | N                          |
| A-30                | $\text{Fe}_3\text{O}_4$                             | 7                                                 | 62                   | 26                               | B, Ca, Mg,<br>P, Na, K           | 7.2             | —                                 | N                          |
| Resistor            |                                                     |                                                   |                      |                                  |                                  |                 |                                   |                            |
| No.                 | Resistor                                            | Noise (dB) Before Durability Test                 |                      |                                  | Noise (dB) After Durability Test |                 |                                   |                            |
|                     |                                                     | 70 d                                              | 30 (MHz)             | 100 (MHz)                        | 200 (MHz)                        | 30 (MHz)        | 100 (MHz)                         | 200 (MHz)                  |
| A-12                | N                                                   | 53                                                | 47                   | 41                               | 57                               | 51              | 46                                |                            |
| A-13                | N                                                   | 52                                                | 46                   | 40                               | 56                               | 50              | 45                                |                            |
| A-14                | N                                                   | 51                                                | 45                   | 41                               | 57                               | 49              | 46                                |                            |
| A-15                | N                                                   | 52                                                | 46                   | 40                               | 56                               | 50              | 45                                |                            |
| A-16                | N                                                   | 52                                                | 47                   | 41                               | 57                               | 51              | 46                                |                            |
| A-17                | N                                                   | 51                                                | 46                   | 41                               | 56                               | 50              | 46                                |                            |
| A-18                | A                                                   | 47                                                | 41                   | 36                               | 49                               | 43              | 38                                |                            |
| A-19                | A                                                   | 45                                                | 40                   | 36                               | 47                               | 42              | 38                                |                            |
| A-20                | A                                                   | 46                                                | 41                   | 35                               | 48                               | 43              | 37                                |                            |
| A-21                | A                                                   | 45                                                | 40                   | 36                               | 47                               | 42              | 38                                |                            |
| A-22                | A                                                   | 45                                                | 40                   | 35                               | 47                               | 42              | 37                                |                            |
| A-23                | A                                                   | 46                                                | 40                   | 35                               | 48                               | 42              | 37                                |                            |
| A-24                | A                                                   | 48                                                | 43                   | 38                               | 50                               | 45              | 40                                |                            |
| A-25                | A                                                   | 48                                                | 42                   | 38                               | 49                               | 44              | 40                                |                            |
| A-26                | A                                                   | 45                                                | 41                   | 35                               | 47                               | 42              | 37                                |                            |
| A-27                | A                                                   | 46                                                | 40                   | 36                               | 47                               | 42              | 38                                |                            |
| A-28                | A                                                   | 47                                                | 41                   | 35                               | 47                               | 42              | 37                                |                            |
| A-29                | N                                                   | 71                                                | 68                   | 62                               | 89                               | 76              | 72                                |                            |
| A-30                | N                                                   | 72                                                | 67                   | 60                               | 86                               | 79              | 71                                |                            |

TABLE 4

| Fe-containing Oxide |                                                     |                                                   |                      |                               |                                  |              |                                   |                            |
|---------------------|-----------------------------------------------------|---------------------------------------------------|----------------------|-------------------------------|----------------------------------|--------------|-----------------------------------|----------------------------|
| No.                 | Composition                                         | Grain Number<br>400 to<br>1,500 ( $\mu\text{m}$ ) | Conductive Substance |                               | Ceramic<br>Elements<br>Contained | Porosity (%) | Protrusion<br>Distance<br>Ld (mm) | Sealing<br>Portion<br>75 d |
|                     |                                                     |                                                   | Coverage (%)         | Thickness T ( $\mu\text{m}$ ) |                                  |              |                                   |                            |
| B-1                 | $\text{SrFe}_{12}\text{O}_{19}$                     | 5                                                 | 49                   | 26                            | Si, B, Mg, Sr                    | 4.7          | —                                 | N                          |
| B-2                 | $\text{FeO}$                                        | 8                                                 | 42                   | 29                            | P, Mg, Ba, Na                    | 4.9          | —                                 | N                          |
| B-3                 | $\text{Ba}_2\text{Co}_2\text{Fe}_{12}\text{O}_{22}$ | 4                                                 | 68                   | 28                            | Ca, Mg, Na, K                    | 5            | —                                 | N                          |
| B-4                 | $(\text{Ni}, \text{Zn})\text{Fe}_2\text{O}_4$       | 7                                                 | 75                   | 27                            | Ca, Ti, Mg, Ba, Li, K            | 5            | —                                 | N                          |

  

| Resistor |                                   |          |           |                                  |          |           |           |  |
|----------|-----------------------------------|----------|-----------|----------------------------------|----------|-----------|-----------|--|
| No.      | Noise (dB) Before Durability Test |          |           | Noise (dB) After Durability Test |          |           |           |  |
|          | 70 d                              | 30 (MHz) | 100 (MHz) | 200 (MHz)                        | 30 (MHz) | 100 (MHz) | 200 (MHz) |  |
| B-1      | N                                 | 70       | 62        | 60                               | 91       | 86        | 82        |  |
| B-2      | N                                 | 69       | 64        | 59                               | 93       | 87        | 81        |  |
| B-3      | N                                 | 68       | 61        | 56                               | 89       | 84        | 80        |  |
| B-4      | N                                 | 68       | 62        | 57                               | 94       | 87        | 81        |  |

In the evaluation tests, 34 types of samples including A-1 to A-30 samples and B-1 to B-4 samples were evaluated. Eleven types of samples from the A-18 to A-28 samples in Table 3 were samples of the spark plug 100d in FIG. 4, and the remaining 23 types of samples were samples of the spark plug 100e in FIG. 7. The 11 types of samples (FIG. 4: the A-18 to A-28 samples) for the spark plug 100d were different from each other in at least one of the protrusion distance Ld and the properties of the magnetic substance structure 200d. The 23 types of samples of the spark plug 100e (illustrated in FIG. 7) were different from each other in the properties of the magnetic substance structure 200d. Tables 2, 3 and 4 illustrate sample numbers, the properties (here, the properties of an iron-containing oxide, the properties of a conductive substance, elements contained in the ceramic, and a porosity) of the magnetic substance structure 200d, the protrusion distance Ld, the existence or non-existence of the sealing portion 75d, the existence or non-existence of the resistor 70d, and noise test results before and after durability tests. The remainder of the configurations of the 34 types of spark plug samples was the same except for the properties of the magnetic substance structure 200d and the configurations of the connection portions 300d and 300e. For example, the magnetic substance structures 200d in the 34 types of samples had substantially the same shape. The magnetic substance structure 200d had an outer diameter (the inner diameter of a portion of the through hole 12d which accommodated the magnetic substance structure 200d) of 3.9 mm.

The composition of the iron-containing oxide, and the number (the number of grains) of specific magnetic grain regions 835 are illustrated as the properties of the iron-containing oxide. The composition of the iron-containing oxide was specified from the iron-containing oxide material contained in the material of the magnetic substance structure 200d. The specific magnetic grain regions 835 used to count the number of grains were the magnetic grain regions 835, the approximate diameter Dc (refer to FIG. 5) of which was in a range of 400  $\mu\text{m}$  or greater and 1,500  $\mu\text{m}$  or less. The approximate diameter Dc was calculated as follows. The magnetic substance structure 200d of each of the samples was cut along a plane including the center axis CL, and the cross-section of the magnetic substance structure 200d was processed using a cross section polisher with which the

cross-section of a specimen was processed using ion beams such as argon ion beams. An image of a region containing a 2.5 mm  $\times$  5.0 mm region corresponding to the target region 800 (refer to FIG. 5) on the cross-section was captured using a scanning electron microscope (SEM). The acceleration voltage of the SEM was set to 15.0 kV, and the working distance was set to a range of 10 mm or greater and 12 mm or less. The SEM images as illustrated in the target region 800 on the center upper side of the FIG. 5 were acquired. The SEM images were binarized using image analysis software (Analysis Five manufactured by Soft Imaging System GmbH). A threshold value for the binarization was set as follows.

(1) An operator defined the position of a grain boundary by confirming a secondary electron image and a backscattered electron image on the SEM image, and drawing a line along a dark boundary (equivalent to the grain boundary) in the backscattered electron image.

(2) In order to improve the backscattered electron image, the operator smoothed the backscattered electron image while maintaining the edge of the grain boundary.

(3) The operator made a graph from the backscattered electron image with the graph showing brightness on the horizontal axis and an incidence on the vertical axis. The obtained graph was a bimodal graph. The brightness of a middle point between two peaks was set as the threshold value for binarization.

The magnetic region 830 and the conductive region 820 (that is, the magnetic grain region 835 and the covering region 825) were separated from each other by the binarization. The area of each of a plurality of magnetic grain regions 835 was calculated using the binarized image. The approximate diameter Dc of each of the plurality of magnetic grain regions 835 was calculated using the calculated area. The number (hereinafter, also referred to as a "specific grain number") of magnetic grain regions 835 having the approximate diameter Dc in a range of 400  $\mu\text{m}$  or greater and 1,500  $\mu\text{m}$  or less was counted. When a portion of one magnetic grain region 835 was protruded out of the target region 800, the one magnetic grain region 835 was treated as one magnetic grain region 835 present in the target region 800 in counting the number of specific magnetic grain regions 835. In a sample with a small specific grain number, the number of magnetic grain region 835 with the approxi-

mate diameter  $D_c$  smaller than the aforementioned range was counted. That is, in a sample with a large specific grain number, the proportion of the magnetic grain region **835** with a large approximate diameter  $D_c$ , that is, the proportion of the magnetic grain region **835** with an approximate diameter  $D_c$  of 400  $\mu\text{m}$  or greater and 1,500  $\mu\text{m}$  or less was high compared to a sample with a small specific grain number.

A coverage and the minimum thickness  $T$  are illustrated as the properties of the conductive substance. The coverage is a proportion of a length of a portion of the edge of the magnetic grain region **835** covered with the covering region **825** to the entire length (the length of one lap) of the edge of the magnetic grain region **835**. The coverage was calculated by analyzing the binarized image. The coverage in the tables is an average value of the coverage of the plurality of magnetic grain regions **835** in the target region **800**. When a portion of the magnetic grain region **835** protruded out of the target region **800**, the coverage was calculated treating the magnetic grain region **835** as one magnetic grain region **835** in the target region **800**. A material selected from the following materials was adopted as the conductive substance: metal (specifically, Ni, Cu, and Fe), perovskite type oxides (specifically,  $\text{LaMnO}_3$ ,  $\text{YMnO}_3$ ), carbon (specifically, carbon black), and carbon compounds (specifically, TiC). In these evaluation tests, the effect of the difference between the conductive substances on noise suppression capability and durability is estimated to be small.

The minimum thickness  $T$  was calculated using the binarized image. When the coverage is less than 100%, the covering region **825** covers only a portion of the edge of the magnetic grain region **835**. An example of the covering region **825** covering a portion of the edge of the magnetic grain region **835** is illustrated on the right upper side of FIG. 5. As illustrated, the covering region **825** covers a portion of the edge of the magnetic grain region **835** from a first end **E1** to a second end **E2**. The thickness of the covering region **825** in the vicinities of the ends **E1** and **E2** may be locally reduced. The minimum thickness  $T$  was calculated using the remainder of the covering region **825** other than end portions **EP1** and **EP2** (in the drawing, the end portions **EP1** and **EP2** were cross-hatched), in which straight distances from the respective ends **E1** and **E2** were less than or equal to a predetermined value (here, 50  $\mu\text{m}$ ).

The elements contained in the ceramic were specified from the elements contained in the ceramic material (in these evaluation tests, an amorphous glass material). The tables illustrate elements other than oxygen. For example, when " $\text{SiO}_2$ " is used as the ceramic material, "Si" without denotation of oxygen (O) is illustrated. Various additive components may be added to the ceramic material. The tables illustrate these additive component elements (for example, Ca and Na). The elements contained in the ceramic can be specified by analyzing the ceramic region **810** using EPMA.

The porosity is a proportion of an area of the pores **812** (refer to FIG. 5) in the remainder of the target region **800** which is other than the magnetic regions **830**. The porosity was calculated as follows. The SEM images were binarized by a similar method as the aforementioned method. A threshold value for binarization was adjusted so that the pores **812** could be separated from other regions. The pores **812** and the other regions were separated from each other by the binarization. The area (referred to as a "first area") of the pores **812** was calculated using the result of the binarization. The area (referred to as a "second area") of the remainder of the target region **800** which was other than the magnetic

regions **830** was calculated using the result of the binarization and the magnetic regions **830** specified by the binarization. The porosity is a proportion of the first area to the second area.

5 The protrusion distance  $L_d$  is the protrusion distance  $L_d$  illustrated in FIG. 6. In the tables, the protrusion distance  $L_d$  of the sample, in which the entirety of the magnetic substance structure **200d** was disposed closer to the leading end direction **D1** side than the rear end **53e** of the metal shell **50**, 10 is not denoted.

With regard to the existence or non-existence of the sealing portion **75d** in the tables, "A" represents that a sample includes the sealing portion **75d**, and "N" represents that a sample does not include the sealing portion **75d**. 15 Similarly, with regard to the existence or non-existence of the resistor **70d**, "A" represents that a sample includes the resistor **70d**, and "N" represents that a sample does not include the resistor **70d**. A sample, in which both the sealing portion **75d** and the resistor **70d** are denoted as "A", are a 20 sample of the spark plug **100d** illustrated in FIG. 4. A sample, in which both the sealing portion **75d** and the resistor **70d** are denoted as "N", are a sample of the spark plug **100e** illustrated in FIG. 7.

An average value of 10 values obtained by analyzing 25 cross-sectional images of the magnetic substance structure **200d** was adopted as, for example, the number of specific magnetic grain regions **835**, the average coverage, the minimum thickness  $T$ , the porosity. Ten cross-sectional images of one type of samples were captured using 10 30 cross-sections of 10 samples of the same type which were manufactured under the same conditions.

In a noise test, a noise intensity was measured according to "automotive—radio noise characteristics—section 2: measurement method of preventive device, current method" 35 of Japanese Automotive Standards Organization D-002-2 (JASO D-002-2). Specifically, the distance of the gap  $g$  of the spark plug sample was adjusted to 0.9  $\text{mm} \pm 0.01 \text{ mm}$ , a voltage in a range of from 13 kV to 16 kV was applied to the sample, and discharge was performed. Current flowing 40 through the terminal metal fixture **40d**, **40e** during discharge was measured using a current probe, and the measured value was converted into the unit of dB. Noise at three types of frequencies, that is, 30 MHz, 100 MHz, and 200 MHz was measured. Each numerical value in the tables denotes a noise 45 intensity with respect to a predetermined reference. As the numerical value increases, the noise intensity also increases. A "before durability test" denotes a noise test result before a durability test, to be described later, is performed, and an "after durability test" entry denotes a noise test result after the durability test is performed. The durability test is a test 50 in which the spark plug samples are discharged with a discharge voltage of 20 kV at a temperature of 200 degrees Celsius for 400 hours. The durability test may cause the progress of the aging of the magnetic substance structure 55 **200d**. A noise intensity "after the durability test" may be higher than a noise intensity "before the durability test" due to the progress of the aging of the magnetic substance structure **200d**.

As illustrated in Tables 2 to 4, as the frequency increased, 60 both of the noise intensities after and before the durability test decreased.

G-2. Regarding Average Coverage of Conductive Substance:

The average coverage of the conductive substance in each 65 of the A-1 to A-6 samples was in a range of 50% or greater and 100% or less. The A-1 to A-6 samples were capable of realizing a sufficiently low noise intensity of 66 dB or less

at all of the frequencies before the durability test. A noise intensity even after the durability test was less than or equal to 77 dB at all of the frequencies, and it was possible to suppress an increase in the noise intensity. That is, it was possible to realize good durability of the magnetic substance structure **200d**. The increased amounts of noise intensity at all of the frequencies induced by the durability test were in a range of 8 dB or greater and 13 dB or less.

The average coverage of the B-1 sample in Table 4 was 49% which was less than the average coverage of each of the A-1 to A-6 samples. Before and after the durability test, the noise intensities of the B-1 sample were higher than those of an arbitrary sample of the A-1 to A-6 samples at the same frequency. The increased amounts of the noise intensity of the B-1 sample induced by the durability test were 21 dB (at 30 MHz), 24 dB (at 100 MHz), and 22 dB (at 200 MHz). The increased amounts of noise intensity of the A-1 to A-6 samples (8 dB or greater and 13 dB or less) were improved by 8 dB or greater than the increased amount of noise intensity of the B-1 sample (21 dB or greater and 24 dB or less) at the same frequency.

The average coverage of the B-2 sample in Table 4 was 42% which was further less than the average coverage of the B-1 sample. Before and after the durability test, the noise intensities of the B-2 sample were higher than those of an arbitrary sample of the A-1 to A-6 samples at the same frequency. The increased amounts of the noise intensity of the B-2 sample induced by the durability test were 24 dB (at 30 MHz), 23 dB (at 100 MHz), and 22 dB (at 200 MHz). The increased amounts of noise intensity of the A-1 to A-6 samples (8 dB or greater and 13 dB or less) were improved by 11 dB or greater than the increased amount of noise intensity of the B-2 sample (22 dB or greater and 24 dB or less) at the same frequency.

As such, the A-1 to A-6 samples with relatively high average coverage were capable of realizing good durability compared to the B-1 and B-2 samples with relatively low average coverage. The estimated reason for this is that when the average coverage is high, the current path formed by the conductive region **820** (refer to FIG. 5) is large, and a large number of current paths are formed by the conductive regions **820** compared to when the average coverage is low.

The average coverage of the conductive substances of the A-1 to A-6 samples suppressing noise and good durability were 50%, 55%, 69%, 72%, 94%, and 100% in an increasing order. A preferable range (range of a lower limit or greater and an upper limit or less) of the average coverage of each of the plurality of magnetic grain regions **835** in the target region **800** can be determined using the aforementioned six values. Specifically, an arbitrary value among the six values can be adopted as the lower limit of the preferable range of the average coverage. An arbitrary value greater than or equal to the lower limit among these values can be adopted as the upper limit. For example, a range of 50% or greater and 100% or less can be adopted as the preferable range of the average coverage of the plurality of magnetic grain regions **835** in the target region **800**.

Typically, when the coverage is greater than or equal to 50%, the covering region **825** is more likely to cover both of a surface of the grain region **835** in a specific direction and a surface thereof in an opposite direction. Accordingly, one covering region **825** is more likely to be in contact with other of the plurality of covering regions **825**. As a result, it is possible to suppress formation of high-resistance portions in the magnetic substance structure **200d** in which electrical resistance is locally high. A large amount of current is generated by current in the high-resistance region compared

to a low-resistance region. The magnetic substance structure **200d** may be aged due to the heat generation. Since the formation of the high-resistance portions is suppressed when the average coverage of the plurality of magnetic grain regions **835** in the target region **800** is greater than or equal to 50%, it is possible to improve the durability of the magnetic substance structure **200d**.

The plurality of magnetic grain regions **835** in the target region **800** may include the magnetic grain regions **835** with average coverage out of the aforementioned preferable range. Also in this case, it is estimated that the spark plug is capable of suppressing noise compared to when the magnetic substance structure **200d** is omitted.

An arbitrary method can be adopted as a method of adjusting the average coverage. For example, it is possible to increase the average coverage by increasing an amount of plating time required to apply non-electrolytic plating to the conductive substance. It is possible to increase the average coverage by increasing the amount of the material of the conductive substance. The average coverage of the 34 types of samples used in these evaluation tests were adjusted as follows. A material powder of magnetic particles, the entire surfaces of which were covered with the conductive substance was prepared. In order to realize an average coverage of 100% or less, a portion of the conductive substance was peeled off from the magnetic particle by stirring the material powder of the magnetic particles covered with the conductive substance.

### G-3. Regarding Ceramic:

The ceramic of the magnetic substance structure **200d** of each of the A-1 to A-6 samples contained at least one of Si, B, and P. The ceramic of the magnetic substance structure **200d** of each of the B-3 and B-4 sample in Table 4 contained Ca, Mg, and K without containing any one of Si, B, and P. The average coverage of the B-3 and B-4 samples were 68% and 75%.

Before the durability test, the noise intensity of each of the A-1 to A-6 samples was the same as or lower than that of an arbitrary sample of the B-3 and B-4 samples at the same frequency. After the durability test, the noise intensity of each of the A-1 to A-6 samples was lower than that of an arbitrary sample of the B-3 and B-4 samples at the same frequency. As such, the A-1 to A-6 samples with the ceramic containing at least one of Si, B, and P was capable of suppressing noise compared to the B-3 and B-4 samples with the ceramic containing none of Si, B, and P.

The increased amounts of noise in the B-3 and B-4 samples induced by the durability test were 21 dB or greater and 26 dB or less. The increased amounts of noise intensity of the A-1 to A-6 samples (8 dB or greater and 13 dB or less) was improved by 8 dB or greater than the increased amounts of noise intensity of the B-3 and B-4 samples at the same frequency.

As such, it was possible to realize good noise suppression capability and good durability by adopting the ceramic containing at least one of Si, B, and P. The estimated reason is as follows. The ceramic containing none of Si, B, and P is more likely to react with the iron-containing oxide due to heat generated by current during discharge compared to the ceramic (for example, glass) containing at least one of Si, B, and P. Accordingly, new phases may be formed by reaction between the ceramic and the iron-containing oxide during the durability test. Accordingly, the number of pores **812** is increased, and the diameter of the pore **812** is increased. In contrast, the ceramic containing at least one of Si, B, and P is a type of glass. When this type of ceramic is used, reaction between Si, B, and P and the iron-containing oxide is

suppressed. Accordingly, an increase in the number of pores **812** and an increase in the diameter of the pore **812** are suppressed compared to when the ceramic containing none of Si, B, and P is used. As a result, it is possible to suppress partial discharge in the pore **812**.

G-4. Regarding Average Coverage and Material of Magnetic Substance Structure **200d**:

The following material were used to manufacture the A-1 to A-6 samples suppressing noise and realizing good durability. A material selected from the following materials was used as the magnetic substances forming the magnetic regions **830** of the magnetic substance structure **200d**: iron oxides ( $Fe_2O_3$ ,  $Fe_3O_4$ , and  $FeO$ ), a spinel ferrite ((Ni, Zn) $Fe_2O_4$ ), and hexagonal ferrites ( $BaFe_{12}O_{19}$  and  $SrFe_{12}O_{19}$ ). The ceramic of the magnetic substance structure **200d** contained at least one of silicon (Si), boron (B), and phosphorous (P).

Typically, in many cases, when the type of a second material is the same as that of a first material, the second material has similar characteristics as those of the first material. Accordingly, it is estimated that even if other materials of the same type are used instead of the aforementioned materials of the magnetic substance structure **200d**, the aforementioned preferable range can be applied to the average coverage of the conductive substance. For example, it is estimated that when the magnetic substance structure **200d** has any one of the following properties Z1 to Z3, the preferable range of the average coverage can be applied.

[Properties Z1] The magnetic substance structure **200d** contains a conductive substance as a conductor.

[Properties Z2] The magnetic substance structure **200d** contains an iron-containing oxide as a magnetic substance.

[Properties Z3] The magnetic substance structure **200d** contains a ceramic containing at least one of silicon (Si), boron (B), and phosphorous (P).

G-5. Regarding Porosity:

The porosity of each of the A-1 to A-6 samples in Table 2 was in a range of 4.3% or greater and 5% or less. As described above, the A-1 to A-6 samples were capable of suppressing noise, and realizing good durability. The porosities of the A-29 and A-30 samples in Table 3 were higher than those of the A-1 to A-6 samples, and were 6.6% and 7.2%, respectively. Other properties of the A-29 and A-30 samples were as follows. That is, the average coverage were 56% and 62%. The ceramic of the magnetic substance structure **200d** contained at least one of Si, B, and P.

Before and after the durability test, the noise intensities of the A-1 to A-6 samples were lower than those of an arbitrary sample of the A-29 and A-30 samples at the same frequency. As such, the A-1 to A-6 samples with relatively low porosities were capable of suppressing noise compared to the A-29 and A-30 samples with relatively high porosities. The estimated reason for this is that when the porosity is low, partial discharge in the pore **812** (refer to FIG. 5) is suppressed compared to when the porosity is high.

The porosities of the A-1 to A-6 samples, the noise suppression capability of which is relatively good, were 4.3%, 4.6%, 4.8%, and 5% in an increasing order. An arbitrary value among these four values can be adopted as the upper limit of a preferable range (range of a lower limit or greater and an upper limit or less) of the porosity. An arbitrary value less than or equal to the upper limit among these values can be adopted as the lower limit. For example, a value in a range of 4.3% or greater and 5% or less can be adopted as the porosity. The noise suppression capability

and the durability are estimated to become better as the porosity becomes lower. Accordingly, 0% may be adopted as the lower limit of the porosity. For example, a range of 0% or greater and 5% or less can be adopted as the preferable range of the porosity.

The noise suppression capability of the A-1 to A-6 samples is good compared to the capability of typical spark plugs (for example, spark plug from which the magnetic substance structure **200d** is omitted). Accordingly, it is estimated that even if the porosity is higher, it is possible to realize practical noise suppression capability. As a result, it is estimated that a higher value (for example, 10%) can be adopted as the upper limit of the porosity. For example, either of the properties of the A-29 sample and the properties of the A-30 sample may be adopted.

An arbitrary method can be adopted as a method of adjusting the porosity. For example, when the firing temperature (heating temperature of the insulator **10d** accommodating the materials of the connection portions **300d** and **300e** in the through hole **12d**) of the magnetic substance structure **200d** is increased, the ceramic material of the magnetic substance structure **200d** is easily melted, and thus it is possible to reduce the porosity. It is possible to block the pores **812** and reduce the porosity by increasing force which is applied to the terminal metal fixtures **40d** and **40e** when the terminal metal fixtures **40d** and **40e** are inserted into the through hole **12d**. It is possible to reduce the porosity by reducing the particle size of the ceramic material of the magnetic substance structure **200d**.

G-6. Regarding Number (Specific Grain Number) of Specific Magnetic Grain Region **835**:

In the A-1 to A-6 samples in Table 2, the specific grain number, that is, the total number of magnetic grain regions **835**, the approximate diameter  $D_c$  of which was in a range of 400  $\mu m$  or greater and 1,500  $\mu m$  or less, were 3 or greater and 5 or less. The specific grain numbers of the A-7 to A-11 samples were greater than those of the A-1 to A-6 samples, and were in a range of 6 or greater and 8 or less. Other properties of the A-7 to A-11 samples were as follows. That is, the average coverage was 56% or greater and 74% or less. The porosity was 4% or greater and 4.3% or less. The ceramic of the magnetic substance structure **200d** contained at least one of Si, B, and P.

Before and after the durability test, the noise intensities of the A-7 to A-11 samples were lower than those of an arbitrary sample of the A-1 to A-6 samples at the same frequency. As such, it was possible to suppress noise when the specific grain number (that is, the number of the magnetic grain regions **835** with relatively large approximate diameters  $D_c$ ) was large compared to when the specific grain number was small. The estimated reason is as follows. A large specific grain number implies that large magnetic substances are disposed in the vicinity of the conductive region **820** (that is, current path). It is possible to suppress noise when large magnetic substances are disposed in the vicinity of the current path (the conductive region **820**) compared to a case when magnetic substances disposed in the vicinity of the current path are small.

The increased amounts of noise of the A-7 to A-11 samples induced by the durability test were 8 dB at all of the frequencies. The increased amounts of noise of the A-1 to A-6 samples were in a range of 8 dB or greater and 13 dB or less, and were greater than the increased amounts of noise of the A-7 to A-11 samples. As such, it was possible to improve the durability of the magnetic substance structure **200d** when the specific grain number was large compared to a case when the specific grain number was small. The

estimated reason is as follows. A large specific grain number implies that the approximate diameter  $D_c$  of the magnetic grain region **835** is large. The large approximate diameter  $D_c$  implies that the covering region **825** or the current path is large. It is possible to improve the durability of the magnetic substance structure **200d** when the current path is large compared to when the current path is small.

As such, in the A-7 to A-11 samples in addition to the A-1 to A-6 samples, it was possible to realize good noise suppression capability and good durability. The specific grain numbers of the A-1 to A-11 samples were 3, 4, 5, 6, 7, and 8 in an increasing order. An arbitrary value among these six values can be adopted as the lower limit of a preferable range (range of a lower limit or greater and an upper limit or less) of the specific grain number. For example, a value greater than or equal to 3 can be adopted as the specific grain number. An arbitrary value greater than or equal to the lower limit among these six values can be adopted as the upper limit. For example, a value less than or equal to 8 can be adopted as the specific grain number.

The specific grain numbers of the A-7 to A-11 samples, in which noise suppression capability and durability were further improved, were 6, 7, and 8 in an increasing order. Accordingly, preferably, the lower limit of the preferable range of the specific grain number is arbitrarily selected from these three values. For example, a value greater than or equal to 6 may be adopted as the specific grain number.

Here, the noise suppression capability and the durability are estimated to become better as the specific grain number becomes larger. Accordingly, it is estimated that a larger value (for example, 20) can be adopted as the upper limit of the specific grain number. The A-12 to A-28 samples realized better noise suppression capability and better durability, which will be described later. The specific grain numbers of the A-1 to A-28 samples were 3, 4, 5, 6, 7, 8, 9, 10, and 11 in an increasing order. An arbitrary value among these nine values can be adopted as the lower limit of a preferable range of the specific grain number. An arbitrary value greater than or equal to the lower limit among these nine values can be adopted as the upper limit. For example, a value less than or equal to 11 may be adopted as the specific grain number.

An arbitrary method can be adopted as a method of adjusting the specific grain number. For example, it is possible to increase the specific grain number by increasing the particle size of the material powder of an iron-containing oxide. Here, the specific grain number may be out of the aforementioned preferable range.

#### G-7. Regarding Minimum Thickness T of Conductive Substance:

The minimum thicknesses T of the A-1 to A-6 samples in Table 2 were less than 1  $\mu\text{m}$ , or 28  $\mu\text{m}$  or greater. The minimum thicknesses T of the A-12 to A-17 samples in Table 3 were 1  $\mu\text{m}$  or greater and 25  $\mu\text{m}$  or less. Other properties of the A-12 to A-17 samples were as follows. That is, the average coverage was 58% or greater and 69% or less. The porosity was 3.6% or greater and 4% or less. The specific grain number was 6 or greater and 9 or less. The ceramic of the magnetic substance structure **200d** contained at least one of Si, B, and P.

Before and after the durability test, the noise intensities of the A-12 to A-17 samples were lower than those of an arbitrary sample of the A-1 to A-6 samples at the same frequency. The estimated reason is as follows. Since the conductive region **820** is thin when the minimum thickness T is less than 1  $\mu\text{m}$ , even before the durability test, the current path may be damaged due to various causes (for example, due to heating during manufacturing or current

during a discharge test). Accordingly, noise may be intensified compared to when the minimum thickness T is large. Since the conductive region **820** is thick when the minimum thickness T is greater than or equal to 28  $\mu\text{m}$ , current may flow through a region positioned away from the magnetic grain region **835**. Accordingly, noise may be intensified compared to when the minimum thickness T is small.

The increased amounts of noise intensity of the A-12 to A-17 samples induced by the durability test were in a range of 4 dB or greater and 6 dB or less. The increased amounts of noise intensity of the A-12 to A-17 samples (4 dB or greater and 6 dB or less) were improved by 3 dB or greater than the increased amounts of noise intensity of the A-1 to A-3 samples (8 dB or greater and 13 dB or less) having the minimum thickness T less than 1  $\mu\text{m}$  at the same frequency. The estimated reason is as follows. When the minimum thickness T is less than 1  $\mu\text{m}$ , the current path is prone to damage. Accordingly, durability may be reduced compared to when the minimum thickness T is large.

The minimum thicknesses T of the A-12 to A-17 samples, in which good noise suppression capability and good durability were realized, were 1  $\mu\text{m}$ , 11  $\mu\text{m}$ , 16  $\mu\text{m}$ , 19  $\mu\text{m}$ , 22  $\mu\text{m}$ , and 25  $\mu\text{m}$  in an increasing order. An arbitrary value among these six values can be adopted as the upper limit of a preferable range (range of a lower limit or greater and an upper limit or less) of the minimum thickness T. An arbitrary value less than or equal to the upper limit among these values can be adopted as the lower limit. For example, a value in a range of 1  $\mu\text{m}$  or greater and 25  $\mu\text{m}$  or less can be adopted as the minimum thickness T. However, as with the A-1 to A-6 samples, the minimum thickness T may be out of the preferable range.

An arbitrary method can be adopted as a method of adjusting the minimum thickness T. For example, when the conductive region **820** is formed by non-electrolytic plating, it is possible to increase the minimum thickness T by increasing an amount of plating time. When a material powder of a conductive substance is used, it is possible to increase the minimum thickness T by increasing the particle sizes of particles of the conductive substance.

#### G-8. Regarding Protrusion Distance Ld:

Unlike other samples, the A-18 to A-28 samples in Table 3 were samples of the spark plug **100d** in FIG. 4, and the protrusion distances Ld (refer to FIG. 6) were greater than zero. Specifically, the protrusion distances Ld of the A-18 to A-23 samples were 10 mm. The protrusion distances Ld of the A-24 to A-28 samples were 1 mm, 3 mm, 5 mm, 7 mm, and 9 mm in the increasing order of the sample numbers. Other properties of the A-18 to A-28 samples were as follows. That is, the average coverage was 69% or greater and 95% or less. The porosity was 3.3% or greater and 3.9% or less. The specific grain number was 8 or greater and 11 or less. The minimum thickness T was 3  $\mu\text{m}$  or greater and 13  $\mu\text{m}$  or less. The ceramic of the magnetic substance structure **200d** contained at least one of Si, B, and P.

Before and after the durability test, the noise intensities of the A-18 to A-28 samples were lower than those of an arbitrary sample of the A-1 to A-17 samples at the same frequency. As illustrated in FIG. 6, the reason for this is that since the capacitance of the capacitor formed by the terminal metal fixture **40d** and the metal shell **50** is reduced when the protrusion distance Ld is large, the flow of electromagnetic noise from the terminal metal fixture **40d** to the metal shell **50** via the insulator **10d** is suppressed.

The protrusion distances Ld of the A-18 to A-28 samples, in which good noise suppression capability were realized, were 1 mm, 3 mm, 5 mm, 7 mm, 9 mm, and 10 mm in an

increasing order. An arbitrary value among these six values can be adopted as the upper limit of a preferable range (range of lower limit or greater and an upper limit or less) of the protrusion distance  $Ld$ . An arbitrary value less than or equal to the upper limit among these values can be adopted as the lower limit. For example, a value in a range of 1 mm or greater and 10 mm or less can be adopted as the protrusion distance  $Ld$ . Noise suppression capability is estimated to become better as the protrusion distance  $Ld$  becomes larger. Accordingly, it is estimated that when the protrusion distance  $Ld$  is greater than zero, that is, when the rear end **200d** of the magnetic substance structure **200d** is positioned closer to the rear end direction **D2** side than the rear end **53e** of the metal shell **50**, noise can be suppressed compared to when the entirety of the magnetic substance structure **200d** is disposed closer to the leading end direction **D1** side than the rear end **53e** of the metal shell **50**. It is estimated that a larger value (for example 20 mm) can be adopted as the upper limit of the protrusion distance  $Ld$ . It is estimated that the aforementioned description regarding the preferable range of the protrusion distance  $Ld$  can be applied to the spark plugs **100**, **100b**, and **100d** including the resistors **70** and **70d**. As with the A-1 to A-17 samples, the entirety of the magnetic substance structure **200d** may be disposed closer to the leading end direction **D1** side than the rear end **53e** of the metal shell **50**.

#### G-9. Regarding Iron-Containing Oxide:

The iron-containing oxides in Table 2 to 4, for example, iron-containing oxides containing at least one of  $FeO$ ,  $Fe_2O_3$ ,  $Fe_3O_4$ , Ni, Mn, Cu, Sr, Ba, Zn, and Y can be adopted as the iron-containing oxide forming the magnetic grain region **830**. It is estimated that iron-containing oxides capable of suppressing electromagnetic noise is not limited to the iron-containing oxides contained in the samples in Table 2 to Table 4, and various types of other iron-containing oxides (for example, various ferrites) can be adopted. The magnetic region **830** may be formed of a plurality of types of iron-containing oxides.

As described above, the configuration of the spark plug (for example, the properties of the magnetic substance structure **200d**) was studied using the samples of the spark plug **100d** (refer to FIG. 4) with the resistor **70d**, and the samples of the spark plug **100e** (refer to FIG. 7) without the resistor **70d**. When the resistor **70d** is omitted, instead of the resistor **70d**, the magnetic substance structure **200d** serves as a resistor suppressing current. Accordingly, it is estimated that a preferable configuration derived from the evaluation results of the samples of the spark plug **100d** (refer to FIG. 4) with the resistor **70d** can be applied to the spark plug **100e** (refer to FIG. 7) without the resistor **70d**. For example, the preferable range of the protrusion distance  $Ld$  may be applied to the spark plug **100e** in FIG. 7. In addition, it is estimated that a preferable configuration derived from the evaluation results of the samples of the spark plug **100e** (refer to FIG. 7) without the resistor **70d** can be applied to the spark plug **100d** (refer to FIG. 4) with the resistor **70d**. For example, the preferable range of the average coverage, the preferable range of the porosity, the preferable range of the specific grain number, the preferable range of the minimum thickness  $T$ , and the preferable material of each of the ceramic region **810**, the conductive region **820**, and the magnetic region **830** may be applied to the spark plug **100d** in FIG. 4.

#### E. Modification Example

(1) The material of the magnetic substances **210** and **210b** is not limited to a MnZn ferrite, and various magnetic

materials can be adopted. For example, various ferromagnetic materials can be adopted. The ferromagnetic material is a material which is spontaneously magnetized. Various materials, for example, materials containing iron oxides such as ferrites (including a spinel type ferrite), and an iron alloy such as alnico (Al—Ni—Co) can be adopted as the ferromagnetic materials. It is possible to appropriately suppress electromagnetic noise by adopting the ferromagnetic material. The material of the magnetic substances **210** and **210b** is not limited to the ferromagnetic materials, and a paramagnetic material may be adopted. It is also possible to suppress electromagnetic noise in this case.

(2) The configuration of the magnetic substance structure is not limited to the configurations illustrated in FIGS. 1 and 2, and various configurations including a magnetic substance and a conductor can be adopted. For example, a coil-shaped conductor may be embedded in a magnetic substance. Typically, a configuration, in which the conductor is connected in parallel with at least a part of the magnetic substance on the conductive path connecting the end of the magnetic substance structure on the leading end direction **D1** side to the end of the magnetic substance structure on the rear end direction **D2** side, is preferably adopted. When such a configuration is adopted, the magnetic substance is capable of suppressing electromagnetic noise. Since the conductor is capable of reducing the end-to-end resistance of the magnetic substance structure, it is possible to suppress an increase in the temperature of the magnetic substance structure. As a result, it is possible to suppress the occurrence of damage to the magnetic substance structure.

Further, as illustrated in FIGS. 4 and 5, the magnetic substance structure may be configured to adopt a member in which a conductive substance as conductor, a magnetic substance, and a ceramic are mixed together. Here, the conductive substance may contain a plurality of types of conductive substances (for example, both of metal and a perovskite type oxide). The magnetic substance may contain a plurality of types of iron-containing oxides (for example, both of  $Fe_2O_3$  and a hexagonal ferrite ( $BaFe_{12}O_{19}$ )). The ceramic may contain a plurality of types of components (for example, both of  $SiO_2$  and  $B_2O_3$ ). In any case, a combination of the conductive substance, an iron-containing oxide as the magnetic substance, and the ceramic is not limited to the combinations of those materials in the samples in Tables 2 and 3, and other various combinations can be adopted. In any case, the composition of the conductive substance and the composition of the iron-containing oxide can be specified by various methods. For example, the compositions may be specified by a micro X-ray diffraction method.

(3) The ceramic contained in the magnetic substance structure **200d** supports the conductive substance and the magnetic substance (iron-containing oxide). Various ceramics can be adopted as the ceramic supporting the conductive substance and the magnetic substance. For example, amorphous ceramic may be adopted. Glass containing one or more components arbitrarily selected from  $SiO_2$ ,  $B_2O_3$ ,  $P_2O_5$ , and the like can be adopted as the amorphous ceramic. Instead, crystalline ceramic may be adopted. Crystallized glass (also referred to as glass ceramic) such as  $Li_2O$ — $Al_2O_3$ — $SiO_2$  glass may be adopted as the crystalline ceramic. In any case, it is estimated that it is possible to realize proper noise suppression capability and proper durability by adopting a ceramic containing at least one of silicon (Si), boron (B), and phosphorous (P) as with the A-1 to A-30 samples in Tables 2 and 3.

(4) It is estimated that various conductive substances can be adopted as the conductive substance forming the con-

ductive region **820** of the magnetic substance structure **200d**. A conductive substance having good oxidation resistance is preferably adopted so as to realize good durability of the magnetic substance structure **200d**. It is possible to suppress aging caused by heat generation resulting from the flow of large current by adopting a conductive substance with an electrical resistivity of  $50\Omega\cdot\text{m}$  or less. For example, a material containing at least one of metal, carbon, a carbon compound, and a perovskite type oxide may be adopted as the material of the conductive region **820**. One or more metals arbitrarily selected from Ag, Cu, Ni, Sn, Fe, Cr, Inconel, a sendust, and a permalloy can be adopted as the metal. One or more compounds arbitrarily selected from  $\text{Cr}_3\text{C}_2$  and TiC can be adopted as the carbon compound.

The perovskite type oxide will be described hereinafter. The perovskite type oxide is represented by general formula  $\text{ABO}_3$ . A leading element A (for example, "La" of  $\text{LaMnO}_3$ ) is an A-site element, and a subsequent element B (for example, "Mn" of  $\text{LaMnO}_3$ ) is a B-site element. When a cubic crystal has a non-distorted crystal structure, a B site is a 6-coordinated site, and is surrounded by an octahedron formed of oxygen. An A site is a 12-coordinated site. One or more oxides arbitrarily selected from 10 oxides, for example,  $\text{LaMnO}_3$ ,  $\text{LaCrO}_3$ ,  $\text{LaCoO}_3$ ,  $\text{LaFeO}_3$ ,  $\text{NdMnO}_3$ ,  $\text{PrMnO}_3$ ,  $\text{YbMnO}_3$ ,  $\text{YMnO}_3$ ,  $\text{SrTiO}_3$ , and  $\text{SrCrO}_3$  can be adopted as such a perovskite type oxide. Since these oxides have low electrical resistance and are stable, it is possible to realize good noise suppression capability and good durability.

It is estimated that it is possible to realize the same level of noise suppression capability and the same level of durability by adopting a plurality of types of perovskite type oxides which have the same A-site element in spite of having different B-site elements. For example, the A-site element of the above-described ten perovskite type oxides is selected from La, Nd, Pr, Yb, Y, and Sr. It is estimated that when the conductive substance of the magnetic substance structure **200d** contains a perovskite type oxide in which the A-site element is at least one of La, Nd, Pr, Yb, Y, and Sr, it is possible to suppress noise, and to realize good durability. An oxide having a plurality of types of A-site elements may be adopted as a perovskite type oxide. The conductive substance may contain a plurality of types of perovskite type oxides.

In any case, elements contained in the conductive region **820** of the magnetic substance structure **200d** can be specified by EPMA analysis.

(5) Instead of the method by which the materials of the magnetic substance structure **200d** are disposed and fired in the through hole **12d** of the insulator **10d**, other arbitrary methods can be adopted to manufacture the magnetic substance structure **200d** illustrated in FIGS. 4, 5, and 7. For example, the materials of the magnetic substance structure **200d** may be molded into a tubular shape using a molding die, and the molded body may be fired to produce a fired magnetic substance structure **200d** having a tubular shape. The fired magnetic substance structure **200d** may be inserted into the through hole **12d** instead of inserting the material powders of the magnetic substance structure **200d** when the through hole **12d** of the insulator **10d** is filled with the material powders of other members (for example, the members **60d**, **70d**, **75d**, and **80d** in FIG. 4, or the members **60e** and **80e** in FIG. 7). It is possible to form the connection portion (for example, the connection portion **300d** in FIG. 4, or the connection portion **300e** in FIG. 7) by inserting the

terminal metal fixtures **40d** and **40e** into the through hole **12d** through the rear opening **14** with the insulator **10d** heated.

(6) The configuration of the magnetic substance structure is not limited to the configurations illustrated in FIGS. 1, 2, 4, 5, and 7, and other various configurations can be adopted. For example, the configurations of the magnetic substance structure **200d** illustrated in FIGS. 4 and 5 may be applied to the magnetic substance structures **200** and **200b** in FIGS. 1 and 2. Members with the same configuration as those of the magnetic substance structures **200d** illustrated in FIGS. 4 and 5 may be adopted as the magnetic substances **210** and **210b** in FIGS. 1 and 2. The configuration of the spark plug **100d** illustrated in FIG. 6 may be applied to the spark plugs **100**, **100b**, and **100e** in FIGS. 1, 2, and 7. For example, the rear end of each of the magnetic substance structures **200**, **200b**, and **200d** in FIGS. 1, 2, and 7 may be positioned closer to the rear end direction **D2** side than the rear end of the metal shell **50**. However, the rear end of each of the magnetic substance structures **200**, **200b**, and **200d** may be positioned closer to the leading end direction **D1** side than the rear end of the metal shell **50**. The configurations of the spark plug **100** and **100b** illustrated in FIGS. 1 and 2 may be applied to the spark plugs **100d** and **100e** in FIGS. 4, 5, and 7. For example, the outer circumferential surface of the magnetic substance structure **200d** illustrated in FIGS. 4 and 7 may be covered with a similar covering portion as the covering portions **290** and **290b** in FIGS. 1 and 2. The magnetic substance structure **200d** may be formed in such a way that the end-to-end resistance of the magnetic substance structure **200d** is in the aforementioned preferable range of the end-to-end resistance of each of the magnetic substance structures **200** and **200b** (for example, is in a range of  $0\Omega$  or greater and  $3\text{k}\Omega$  or less, or in a range of  $0\Omega$  or greater and  $1\text{k}\Omega$  or less). However, the end-to-end resistance of the magnetic substance structure **200d** may be out of the aforementioned preferable range. At least one of the resistors **70** and **70d**, and the sealing portions **60**, **60d**, **60e**, **75**, **75b**, **75d**, **80**, **80b**, **80d**, and **80e** may contain crystalline ceramic. The magnetic substance structure **200d** may be disposed closer to the leading end direction **D1** side than the resistor **70d**. At least one of the sealing portions **60**, **60d**, **60e**, **75**, **75b**, **75d**, **80**, **80b**, **80d**, and **80e** may be omitted.

(7) The configuration of the spark plug is not limited to the configurations illustrated in FIGS. 1 and 2, Table 1, FIGS. 4 to 7, and Tables 2 to 4, and various configurations can be adopted. For example, a noble metal tip may be provided in a portion of the center electrode **20** in which the gap **g** is formed. A noble metal tip may be provided in a portion of the ground electrode **30** in which the gap **g** is formed. An alloy containing noble metal such as iridium or platinum can be adopted as the material of the noble metal tip.

In the embodiments, the leading end portion **31** of the ground electrode **30** faces the leading end surface **20s1** facing the leading end direction **D1** side of the center electrode **20** to form the gap **g**. Instead, the leading end portion of the ground electrode **30** may face the outer circumferential surface of the center electrode **20** to form a gap.

The present invention has been described based on the embodiments and the modification examples; however, the embodiments of the invention are given to help easy understanding of the present invention, and do not limit the present invention. The present invention can be modified

and improved insofar as the modification and the improvements do not depart from the purport and the claims of the present invention.

## INDUSTRIAL APPLICABILITY

This disclosure can be suitably used in a spark plug of an internal combustion engine or the like.

## REFERENCE SIGNS LIST

- 5: gasket
- 6: first rear end-side packing
- 7: second rear end-side packing
- 8: front end-side packing
- 9: talc
- 10, 10c, 10d: insulator (ceramic insulator)
- 10i: inner circumferential surface
- 11: second reduced outer diameter portion
- 12, 12c, 12d: through hole (axial hole)
- 13: leg portion
- 14: rear opening
- 15: first reduced outer diameter portion
- 16: reduced inner diameter portion
- 17: leading end side trunk portion
- 18: rear end-side trunk portion
- 19: flanged portion
- 20: center electrode
- 20s1: leading end surface
- 21: electrode base member
- 22: core member
- 23: head portion
- 24: flanged portion
- 25: leg portion
- 30: ground electrode
- 31: leading end portion
- 35: base member
- 36: core
- 40, 40c, 40d, 40e: terminal metal fixture
- 41: cap installation portion
- 42: flanged portion
- 43, 43c, 43d, 43e: leg portion
- 50: metal shell
- 51: tool engagement portion
- 52: screw portion
- 53: crimped portion
- 54: seat portion
- 55: trunk portion
- 56: reduced inner diameter portion
- 58: deformed portion
- 59: through hole
- 60, 60d, 60e: first conductive sealing portion
- 70, 70d: resistor
- 75, 75b, 75c, 75d, 80e: second conductive sealing portion
- 80, 80b, 80d: third conductive sealing portion
- 100, 100b, 100c, 100d, 100e: spark plug
- 200, 200b, 200d: magnetic substance structure
- 210, 210b: magnetic substance
- 220, 220b: conductor
- 290, 290b: covering portion
- 300, 300b, 300c, 300d, 300e: connection portion
- 800: target region
- 810: ceramic region
- 812: pore
- 812, 820: conductive region
- 825: covering region
- 825, 830: magnetic region

- 835: magnetic grain region
- 840: composite grain region
- g: gap
- CL: center axis (axial line)

Having described the invention, the following is claimed:

1. A spark plug comprising:  
an insulator having a through hole extending in a direction of an axial line;  
a center electrode, at least a part of which is inserted into a leading end side of the through hole;  
a terminal metal fixture, at least a part of which is inserted into a rear end side of the through hole; and  
a connection portion connecting the center electrode and the terminal metal fixture together in the through hole, wherein the connection portion includes:  
a resistor; and  
a magnetic substance structure including a magnetic substance and a conductor and being disposed on a leading end side or a rear end side of the resistor while being positioned away from the resistor, and wherein, among the resistor and the magnetic substance structure, when a member disposed on a leading end side is defined as a first member and a member disposed on a rear end side is defined as a second member, the connection portion further includes:  
a first conductive sealing portion that is disposed on a leading end side of the first member and is in contact with the first member;  
a second conductive sealing portion that is disposed between the first member and the second member and is in contact with the first member and the second member; and  
a third conductive sealing portion that is disposed on a rear end side of the second member and is in contact with the second member,  
wherein the magnetic substance structure contains:  
(1) a conductive substance as the conductor;  
(2) an iron-containing oxide as the magnetic substance; and  
(3) a ceramic containing at least one of silicon (Si), boron (B), and phosphorous (P),  
wherein, in a cross-section of the magnetic substance structure including the axial line, when a target region is defined as a rectangular region having the axial line as a center line, a side of 2.5 mm in a direction perpendicular to the axial line, and a side of 5.0 mm in the direction of the axial line,  
a region of the iron-containing oxide includes a plurality of grain-shaped regions in the target region, at least a part of an edge of each of the plurality of grain-shaped regions is covered with the conductive substance in the target region, and  
when a coverage is defined as a proportion of a length of a portion of the edge of the grain-shaped region covered with the conductive substance to an entire length of the edge of the grain-shaped region, an average value of the coverage of the plurality of grain-shaped regions is greater than or equal to 50% in the target region, and  
wherein, in the target region in the cross-section of the magnetic substance structure, a total number of grain-shaped regions, an area of which is the same as an area of a circle with a diameter in a range of 400  $\mu\text{m}$  or greater and 1,500  $\mu\text{m}$  or less, is greater than or equal to 6.

45

2. The spark plug according to claim 1, wherein an electrical resistance between a leading end and a rear end of the magnetic substance structure is less than or equal to 3 kΩ.
3. The spark plug according to claim 2, wherein the electrical resistance between the leading end and the rear end of the magnetic substance structure is less than or equal to 1 kΩ.
4. The spark plug according to claim 1, wherein the conductor includes a spiral coil surrounding at least a part of an outer circumference of the magnetic substance, and wherein an electrical resistance of the coil is less than an electrical resistance of the magnetic substance.
5. The spark plug according to claim 1, wherein the conductor includes a conductive portion penetrating through the magnetic substance in the direction of the axial line.
6. The spark plug according to claim 1, wherein the magnetic substance structure is disposed on the rear end side of the resistor.
7. The spark plug according to claim 1, wherein the connection portion further includes a covering portion that covers at least a part of an outer surface of the magnetic substance structure while being interposed between the magnetic substance structure and the insulator.
8. The spark plug according to claim 1, wherein the magnetic substance is made of a ferromagnetic material containing an iron oxide.
9. The spark plug according to claim 8, wherein the ferromagnetic material is a spinel type ferrite.
10. The spark plug according to claim 1, wherein the magnetic substance is a NiZn ferrite or a MnZn ferrite.
11. The spark plug according to claim 1, wherein, in the target region in the cross-section of the magnetic substance structure, a porosity of a remainder of the target region other than the region of the iron-containing oxide is less than or equal to 5%.
12. The spark plug according to claim 1, wherein, in the target region in the cross-section of the magnetic substance structure, a minimum thickness of the conductive substance covering the edge of the grain-shaped region is 1 μm or greater and 25 μm or less.
13. The spark plug according to claim 1, further comprising:
  - a metal shell disposed on a radial circumference of the insulator,

46

wherein the magnetic substance structure is disposed on the rear end side of the resistor, and wherein a rear end of the magnetic substance structure is positioned closer to the rear end side than a rear end of the metal shell.

14. A spark plug comprising:  
 an insulator having a through hole extending in a direction of an axial line;  
 a center electrode, at least a part of which is inserted into a leading end side of the through hole;  
 a terminal metal fixture, at least a part of which is inserted into a rear end side of the through hole; and  
 a connection portion connecting the center electrode and the terminal metal fixture together in the through hole, wherein the connection portion includes a magnetic substance structure including a magnetic substance and a conductor,  
 wherein the magnetic substance structure contains:  
 (1) a conductive substance as the conductor;  
 (2) an iron-containing oxide as the magnetic substance;  
 and  
 (3) a ceramic containing at least one of silicon (Si), boron (B), and phosphorous (P),  
 wherein, in a cross-section of the magnetic substance structure including the axial line, when a target region is defined as a rectangular region having the axial line as a center line, a side of 2.5 mm in a direction perpendicular to the axial line, and a side of 5.0 mm in the direction of the axial line,  
 a region of the iron-containing oxide includes a plurality of grain-shaped regions in the target region, at least a part of an edge of each of the plurality of grain-shaped regions is covered with the conductive substance in the target region, and  
 when a coverage is defined as a proportion of a length of a portion of the edge of the grain-shaped region covered with the conductive substance to an entire length of the edge of the grain-shaped region, an average value of the coverage of the plurality of grain-shaped regions is greater than or equal to 50% in the target region, and  
 wherein, in the target region in the cross-section of the magnetic substance structure, a total number of grain-shaped regions, an area of which is the same as an area of a circle with a diameter in a range of 400 μm or greater and 1,500 μm or less, is greater than or equal to 6.

\* \* \* \* \*